



US010975312B2

(12) **United States Patent**  
**Lin et al.**

(10) **Patent No.:** **US 10,975,312 B2**  
(b4) **Date of Patent:** **Apr. 13, 2021**

(54) **PROCESS FOR ONE-POT LIQUEFACTION OF BIOMASS OR COAL AND BIOMASS**

(71) Applicant: **BEIJING SANJU ENVIRONMENTAL PROTECTION & NEW MATERIALS CO., LTD,**  
Beijing (CN)

(72) Inventors: **Ke Lin**, Beijing (CN); **Lin Li**, Beijing (CN); **Lixin Guo**, Beijing (CN)

(\*) Notice: Subject to any disclaimer, the term of this patent is extended or adjusted under 35 U.S.C. 154(b) by 0 days.

(21) Appl. No.: **16/537,527**

(22) Filed: **Aug. 10, 2019**

(65) **Prior Publication Data**

US 2019/0359892 A1 Nov. 28, 2019

**Related U.S. Application Data**

(63) Continuation of application No. PCT/CN2018/122665, filed on Dec. 21, 2018.

(30) **Foreign Application Priority Data**

Dec. 25, 2017 (CN) ..... 201711419221.2  
Dec. 25, 2017 (CN) ..... 201711420263.8  
Dec. 25, 2017 (CN) ..... 201711420278.4  
Dec. 25, 2017 (CN) ..... 201711421720.5  
Dec. 26, 2017 (CN) ..... 201711429908.4  
Dec. 26, 2017 (CN) ..... 201711430518.9

(51) **Int. Cl.**

**C10G 1/06** (2006.01)  
**C10L 1/32** (2006.01)

(52) **U.S. Cl.**

CPC ..... **C10G 1/06** (2013.01); **C10L 1/32** (2013.01); **C10G 2300/1014** (2013.01); **C10L 2200/0484** (2013.01); **C10L 2290/544** (2013.01)

(58) **Field of Classification Search**

CPC combination set(s) only.  
See application file for complete search history.

(56) **References Cited**

U.S. PATENT DOCUMENTS

8,623,102 B2 1/2014 Quignard et al.  
2011/0167713 A1 7/2011 Quignard et al.  
2017/0362416 A1\* 12/2017 Srinivasan ..... C08L 9/06  
2018/0023014 A1 1/2018 Li

FOREIGN PATENT DOCUMENTS

|    |             |         |
|----|-------------|---------|
| CA | 1294236 C   | 1/1992  |
| CN | 1544580 A   | 11/2004 |
| CN | 101805629 A | 8/2010  |
| CN | 101899314 A | 12/2010 |
| CN | 102443130 A | 5/2012  |
| CN | 103148498 A | 6/2013  |
| CN | 103242871 A | 8/2013  |

|    |               |         |
|----|---------------|---------|
| CN | 104927948 A   | 9/2015  |
| CN | 104962331 A   | 10/2015 |
| CN | 106967469 A   | 7/2017  |
| CN | 108251150 A   | 12/2017 |
| CN | 108085042 A   | 5/2018  |
| CN | 108219818 A   | 6/2018  |
| CN | 108219819 A   | 6/2018  |
| CN | 108264916 A   | 7/2018  |
| CN | 108264920 A   | 7/2018  |
| EP | 0182309 A     | 11/1984 |
| WO | 2016124148 A1 | 8/2016  |

**OTHER PUBLICATIONS**

European Search Report of European Patent Application No. 18896217. 9.

Second Office Action of Chinese Application No. 2017114217205. Internation Search Report of PCT/CN2018/122665, dated Mar. 26, 2019.

Priority Document CN2017114217205\_Decision of Refusal dated Nov. 13, 2019.

Written Opinion of PCT/CN2018/122665, dated Mar. 26, 2019.

OA1 of priority CN2017114217205, dated Mar. 9, 2019.

OA1 of priority CN2017114305189, dated Mar. 8, 2019.

OA1 of priority CN2017114202784, dated Mar. 18, 2019.

OA1 of priority CN2017114299084, dated Jan. 31, 2019.

OA1 of priority CN2017114192212, dated Mar. 15, 2019.

OA1 of priority CN2017114202638, dated Mar. 8, 2019.

OA1 of priority CN2017114202638, dated May 20, 2019.

OA2 of priority CN2017114299084, dated Mar. 20, 2019.

OA2 of priority CN2017114202638, dated May 10, 2019.

“Research progress and prospects of biomass solidification briquetting technology” 74 Engineering Sciences.

Decision of Rejection of priority CN2017114299084, dated May 30, 2019.

Decision of Rejection of priority CN2017114202638, dated Aug. 9, 2019.

(Continued)

*Primary Examiner* — Ellen M McAvoy

*Assistant Examiner* — Chantel L Graham

(74) *Attorney, Agent, or Firm* — W&K IP

(57) **ABSTRACT**

Disclosed is a process for the one-pot liquefaction of a biomass or coal and a biomass, the process comprising: first preparing a slurry containing a catalyst, a vulcanizing agent and a biomass (and coal), and then introducing hydrogen gas into the slurry to carry out a reaction. Preparing the slurry comprises: subjecting a biomass (and coal) sequentially to drying, a first pulverization, compression and a second pulverization, then mixing same with a catalyst and a vulcanizing agent to obtain a mixture, and adding the mixture to an oil product for grinding and pulping to obtain a biomass slurry. By means of the treatment process of subjecting the straw firstly to compression and then to a second pulverization, the volume of the straw is greatly reduced, thereby facilitating the dispersion thereof in the oil product.

(56)

**References Cited**

OTHER PUBLICATIONS

OA3 of priority CN2017114217205, dated Aug. 15, 2019.  
OA2 of priority CN2017114305189, dated Aug. 21, 2019.  
OA2 of priority CN2017114192212, dated Aug. 21, 2019.  
Subcritical Supercritical Water Technique and Principle, 2014.  
First Office Action of European Patent Application No. 18896217.9.

\* cited by examiner

## 1

PROCESS FOR ONE-POT LIQUEFACTION  
OF BIOMASS OR COAL AND BIOMASSCROSS-REFERENCE TO RELATED  
APPLICATIONS

This application is a continuation of International Patent Application No. PCT/CN2018/122665 with an international filing date of Dec. 21, 2018, designating the United States, now pending, and further claims priority benefits to Chinese Patent Applications No. 201711421720.5, filed on Dec. 25, 2017, Chinese Patent Applications No. 201711420278.4, filed on Dec. 25, 2017, Chinese Patent Applications No. 20171111419221.2, filed on Dec. 25, 2017, Chinese Patent Applications No. 201711420263.8, filed on Dec. 25, 2017, Chinese Patent Applications No. 201711430518.9, filed on Dec. 26, 2017, and Chinese Patent Applications No. 201711429908.4, filed on Dec. 26, 2017. The contents of all of the aforementioned applications, including any intervening amendments thereto, are incorporated herein by reference.

## TECHNICAL FIELD

The present invention relates to the technical field of biological energy conversion, and particularly to a process for one-pot liquefaction of biomass or coal and biomass.

## BACKGROUND

With rapid development of the social economy, the non-renewable fossil energy, such as coal, crude oil, natural gas, oil shale, etc., is exhausted gradually, and environmental pollution caused by contaminants, such as  $\text{CO}_2$ ,  $\text{SO}_2$ ,  $\text{NO}_x$ , etc., generated after the fossil non-renewable energy is burnt, is increasingly serious, so that the human beings have to seriously consider energy access ways and environment improvement methods. Biomass is a renewable energy, which has huge potential and advantages in the aspects of meeting energy demands, reducing environment pollution and improving energy structure. Biomass refers to all organic substances formed by directly or indirectly using the photosynthesis of green plants, including plants, animals, microorganisms and excretions and metabolites thereof, and biomass has renewability, low pollution and wide distribution. In recent years, conversion and utilization of biomass energy are developing towards high efficiency and cleanliness, and biomass liquefaction technology is one of the important points. The liquefaction mechanism is as follows: biomass is firstly pyrolyzed into oligomers, and then subjected to dehydration, dehydroxylation, dehydrogenation, deoxygenation and decarboxylation to form small molecule compounds, which are then subjected to reactions such as condensation, cyclization, polymerization, etc. to form new compounds. The existing biomass liquefaction process mainly comprises indirect liquefaction and direct liquefaction. Direct liquefaction is to directly liquefy solid biomass to liquid by carrying out hydrolysis and supercritical liquefaction or introducing hydrogen, inert gas, etc. under a suitable temperature and a suitable pressure in the presence of a solvent or a catalyst. Biomass direct liquefaction process mainly comprises pyrolysis liquefaction, catalytic liquefaction, pressurized hydroliquefaction, etc., among which pressurized hydroliquefaction has high products yield and good quality. Pressurized hydroliquefaction generally comprises complex procedures, such as solid material drying, crushing, slurry preparing, heating, pressurizing, reacting,

## 2

ing, separating, etc. For example, Chinese patent application CN103242871A discloses a heavy oil and biomass hydrogenation co-liquefaction treatment process, which comprises pre-pulverizing a dried biomass to 40-100-mesh and mixing it with a heavy oil to form a slurry, adding a catalyst and a vulcanizing agent into the slurry, placing the resulted mixture in a slurry bed hydrogenation reactor to undergo hydrogenation and thermal cracking reactions under a temperature of 370-430° C. and a hydrogen partial pressure of 4-8 MPa, and fractioning the reaction product, thereby obtaining a bio-oil and coke.

The above-mentioned process realizes the conversion of biomass to bio-oil, but in the above technique there are some problems. In one respect, the slurry formed from biomass and heavy oil needs to be pumped to the slurry bed hydrogenation reactor. However, most biomass (for example straw) has low specific gravity due to its abundant porosity, making it difficult to dissolve in the biomass liquefaction solvent, resulting in lower concentration of biomass in the slurry (the biomass in the above technology only accounts for 5-20 wt % of the mass of the heavy oil), which results in a limited amount of biomass transport per unit time, thus, the above hydrogenation co-liquefaction process has lower production efficiency, higher industrial costs, and higher energy consumption. In another respect, biomass with porosity is easy to float on the surface of the liquefied solvent, furthermore, heavy oil used as a slurry solvent has large viscosity, making the slurry being difficult to flow, which easily causes blockage of the conveying pipe, so it is difficult to achieve smooth transportation by the pump. Although in the prior art, researchers attempt to add dispersing agent to the slurry to increase the concentration and dispersion of biomass in the slurry, but the adding of dispersing agent often affects the quality of the bio-oil. In addition, the biomass has a low conversion rate in the above technology (the conversion rate is only about 90%). Therefore, a technical problem to be urgently solved by those skilled in the art is to improve the existing biomass liquefaction process so as to increase the concentration of biomass in the slurry, increase the pumping capacity of the biomass per unit time, achieve smooth pumping, reduce energy consumption, and increase biomass conversion rate.

## SUMMARY OF THE INVENTION

Therefore, the present invention aims to overcome the problems of low biomass transport by the pumps, unstable transportation, low biomass conversion rate and high energy consumption in the prior biomass liquefaction process, and further to provide a process for one-pot liquefaction of biomass or coal and biomass.

For this purpose, the above-mentioned object of the present invention is achieved by the following technical solutions:

In one aspect, the present invention provides a first technical solution for one-pot liquefaction process for biomass, comprising the following steps:

preparing a slurry containing a catalyst, a vulcanizing agent and a biomass, and introducing hydrogen into the slurry to carry out a reaction under a pressure of 15-25 MPa and a temperature of 380-480° C., thereby obtaining a bio-oil;

wherein, the slurry is prepared with using straw as the biomass according to the following steps: subjecting the straw sequentially to drying, a first pulverization, compression and a second pulverization to obtain a pretreated biomass, and then mixing the pretreated biomass with the

catalyst and the vulcanizing agent to obtain a mixture, and adding the mixture to an oil to carry out grinding pulping to obtain the slurry having a straw concentration of 30 wt % to 60 wt %.

The straw raw material in the present invention can be selected from the group consisting of straw of cereal crops, such as wheat, rice, corn, reed, sorghum, millet, etc., and can also be straw of leguminous plants such as soybean, adzuki bean, mung bean, broad bean, pea, etc., and can also be straw of fiber crops, such as cotton, flax, ramie, and any combination thereof.

Said subjecting the straw to compression is carried out under a pressure of 0.5-3 MPa and a temperature of 30-60° C.

Said subjecting the straw to drying is carried out at a temperature of 50-70° C. for a period of 3-5 h to obtain a dried straw having a moisture content of less than 2 wt %, and after the first pulverization the dried straw has a median particle size of 100-300  $\mu\text{m}$ , and after the second pulverization the dried straw has a median particle size of 30-50  $\mu\text{m}$  and a bulk density of 400-500  $\text{kg/m}^3$ .

The slurry has a viscosity of 500-1400  $\text{mPa}\cdot\text{s}$  (50° C.).

The slurry has a straw content of 55-60 wt %.

The oil is selected from the group consisting of waste animal and vegetable oil, waste mineral oil, mineral oil, distillate oil, and any combination thereof.

Further, the waste animal and vegetable oil is selected from the group consisting of gutter oil, hogwash oil, sour oil, and any combination thereof.

The waste mineral oil is a waste lubricating oil and/or a waste engine oil.

The mineral oil is selected from the group consisting of heavy oil, residual oil, anthracene oil, washing oil, and any combination thereof.

The grinding pulping is stirring pulping, dispersing pulping, emulsifying pulping, shearing pulping, or homogeneous pulping.

The catalyst is selected from the group consisting of amorphous FeOOH, amorphous alumina loading an active component, biomass charcoal loading an active component, and any combination thereof, and wherein the active component is selected from the group consisting of oxides of metals of group VIB, group VIIB, group VIII, and any combination thereof in the periodic table of elements.

The active component is selected from the group consisting of oxides of Mo, W, Fe, Co, Ni, Mn, Pd and any combination thereof.

The catalyst is present in an amount of 1-10 wt %, preferably 1-4 wt % of the mass of the pretreated biomass, and has a particle size of 5-500  $\mu\text{m}$ ; and the vulcanizing agent is present in an amount of 0.1-0.4 wt % of the mass of the pretreated biomass.

Said introducing hydrogen into the slurry comprises: introducing a high-pressure hydrogen into the slurry to prepare a reaction raw material mixture, wherein the high-pressure hydrogen and the slurry have a volume ratio of (600-1500):1; and heating the reaction raw material mixture to 380-480° C. and feeding it into a slurry bed reactor to undergo hydrolysis, cracking and hydrogenation reactions, and simultaneously introducing a cold hydrogen into the slurry bed reactor by controlling the slurry bed reactor to have a total gas velocity of 0.02-0.2 m/s, preferably 0.05-0.08 m/s; wherein, the high-pressure hydrogen has a pressure of 13-25 MPa, and the cold hydrogen has a temperature of 60-135° C.

Said introducing the high-pressure hydrogen into the slurry comprises two steps of: firstly, introducing a high-

pressure hydrogen into the slurry till the volume ratio of the high-pressure hydrogen to the slurry is (50-200):1, and heating the slurry to 200-350° C., and secondly, introducing a high-pressure hydrogen into the slurry.

5 The cold hydrogen is injected via 3-5 injection ports which are sequentially formed in a height direction in a side wall of the slurry bed reactor.

The catalyst stored in the slurry bed reactor is controlled in an amount of 5-30 wt % of the mass of liquid phase in the 10 slurry bed reactor; and the reaction is carried out for a period of 30-120 min.

The biomass charcoal loading with an active component is prepared by a method comprising: S1, carrying out acidification or alkalization on biomass charcoal to produce 15 a biomass charcoal support; and S2, mixing the biomass charcoal support with an active component, followed by grinding to produce the biomass charcoal loading the active component.

The active component is selected from the group consisting of oxides of Mo, W, Fe, Co, Ni, Mn, Pd, and any combination thereof, and based on mass of metal elements, the active component accounts for 1-5% of the mass of the biomass charcoal support.

Said mixing and grinding the biomass charcoal support with an active component comprises the steps of: carrying out vibration grinding and/or plane grinding and/or ball milling on the active component and the biomass charcoal support, thereby obtaining the biomass charcoal loading the active component and having a particle size of 5-500  $\mu\text{m}$ .

The acidification is carried out with an acid medium which has a  $\text{H}^+$  concentration of 0.5-5 mol/L. A volume ratio of the carbonized biomass charcoal to the acid medium is (1:5)-(1:15). The acidification is carried out at a temperature of 30-80° C. for a period of 1-10 h. The alkalization is carried out with an alkaline medium which has an  $\text{OH}^-$  concentration of 0.5-5 mol/L. A volume ratio of the carbonized biomass charcoal to the alkaline medium is (1:5)-(1:15). The alkalization is carried out at a temperature of 30-80° C. for a period of 1-10 h.

40 The vulcanizing agent can be sulfur, carbon disulfide or dimethyl disulfide.

In a second aspect, the present invention also provides a second technical solution for one-pot liquefaction process for biomass, comprising the following steps:

45 preparing a slurry containing a catalyst, a vulcanizing agent and a biomass, and introducing hydrogen into the slurry to carry out a reaction under a pressure of 13-25 MPa and a temperature of 300-500° C., thereby obtaining a bio-oil.

The catalyst comprises amorphous alumina loading a first active component, or biomass charcoal loading a first active component, wherein the first active component is selected from the group consisting of oxides of metals of group VIB, group VIIB, group VIII, and any combination thereof in the 50 periodic table of elements.

The catalyst further comprises amorphous FeOOH, and/or biomass charcoal loading a second active component, wherein the second active component is selected from the group consisting of oxides of Mo, W, Fe, Co, Ni, Pd, and any combination thereof. The catalysts can be either used alone or used in combination. When used in combination, a mass ratio of the iron oxyhydroxide to the biomass charcoal loading a second active component is 0.5-5.

55 The vulcanizing agent specifically can be but not limited to sulfur or dimethyl sulfide. Any compound capable of converting the active component in the catalyst from oxides into corresponding sulfides can be taken as the vulcanizing

## 5

agent. In the present invention, the vulcanizing agent is present in an amount of 4-10 wt % of the mass of the catalyst.

The slurry has a biomass content of 10-50 wt %, preferably 30-40 wt %.

The catalyst is present in an amount of 1-10 wt %, preferably 1-4 wt % of the mass of the biomass, and has a particle size of 5-500  $\mu\text{m}$ .

The slurry is prepared by:

adding the catalyst and the vulcanizing agent respectively into a liquid biomass to form the slurry, wherein the liquid biomass is selected from the group consisting of vegetable oil, animal oil, gutter oil, animal wastes, and any combination thereof; or

drying, pulverizing and removing dust from a solid biomass, followed by mixing with a catalyst and a vulcanizing agent to obtain a mixture; and adding the mixture to an oil to form a slurry, wherein the oil is selected from the group consisting of vegetable oil, animal oil, coal tar, petroleum, the bio-oil prepared by the process in the present invention, and any combination thereof.

The solid biomass raw material can be straw of crops, such as wheat, rice, corn, cotton, etc., or industrial crops, such as reed, pennisetum sinese, trees, tree leaves, melons, fruits, vegetables, etc., or algae, industrial wood and paper wastes, etc.; and the solid biomass raw material may be one biomass, or a biomass raw material consisting of various biomass.

The dried solid biomass has a moisture content of 3-15 wt %, preferably 5-10 wt %; and the pulverized solid biomass has a particle size of 1-5000  $\mu\text{m}$ , preferably 20-1500  $\mu\text{m}$ .

Said introducing hydrogen into the slurry comprises:

introducing a high-pressure hydrogen into the slurry to prepare a reaction raw material mixture, wherein the high-pressure hydrogen and the slurry have a volume ratio of (600-1500):1; and

heating the reaction raw material mixture to 320-450° C. and feeding it into a slurry bed reactor to undergo hydrolysis, cracking and hydrogenation reactions, and simultaneously introducing a cold hydrogen into the slurry bed reactor by controlling the slurry bed reactor to have a total gas velocity of 0.02-0.2 m/s, preferably 0.05-0.08 m/s;

wherein, the high-pressure hydrogen has a pressure of 13-27 MPa, and the cold hydrogen has a temperature of 60-135° C.

Said introducing the high-pressure hydrogen into the slurry comprises two steps of:

firstly, introducing a high-pressure hydrogen into the slurry till the volume ratio of the high-pressure hydrogen to the slurry is (50-200):1, and heating the slurry to 200-350° C., and

secondly, introducing a high-pressure hydrogen into the slurry.

The cold hydrogen is injected via 3-5 injection ports which are sequentially formed in a height direction in a side wall of the slurry bed reactor.

The catalyst stored in the slurry bed reactor is controlled in an amount of 5-30 wt % of the mass of liquid phase in the slurry bed reactor; and the reaction is carried out for a period of 15-90 min.

The biomass charcoal loading a second active component is prepared by:

S1, carrying out acidification or alkalization on carbonized biomass charcoal to produce a biomass charcoal support; and

## 6

S2, mixing the biomass charcoal support with a second active component, followed by grinding to produce a biomass charcoal loading a second active component.

The second active component is selected from the group consisting of oxides of Mo, W, Fe, Co, Ni and Pd, and based on mass of metal elements, the second active component accounts for 1-5 wt % of the mass of the second biomass charcoal support.

Said mixing and grinding the second biomass charcoal support with the second active component comprises: carrying out vibration grinding and/or plane grinding and/or ball milling on the second active component and the second biomass charcoal support, thereby obtaining biomass charcoal loading a second active component and having a particle size of 5-500  $\mu\text{m}$ .

The acidification is carried out with an acid medium which has a  $\text{H}^+$  concentration of 0.5-5 mol/L. A volume ratio of the carbonized biomass charcoal to the acid medium is (1:5)-(1:15), and the acidification is carried out at a temperature of 30-80° C. for a period of 1-10 h. The alkalization is carried out with an alkaline medium which has an  $\text{OH}^-$  concentration of 0.5-5 mol/L. A volume ratio of the carbonized biomass charcoal to the alkaline medium is (1:5)-(1:15), and the alkalization is carried out at a temperature of 30-80° C. for a period of 1-10 h.

In a third aspect, the present invention also provides a third technical solution for one-pot liquefaction process for biomass, comprising the following steps:

preparing a slurry containing a catalyst, a vulcanizing agent and a biomass, and introducing hydrogen into the slurry to carry out a reaction under a pressure of 15-25 MPa and a temperature of 380-480° C., thereby obtaining a bio-oil.

The slurry is prepared with using a vegetable oil residue as the biomass according to the following steps: subjecting the vegetable oil residue sequentially to drying, a first pulverization, compression and a second pulverization to obtain a pretreated biomass, and then mixing the pretreated biomass with the catalyst and the vulcanizing agent to obtain a mixture, and adding the mixture to an oil to carry out grinding pulping to obtain the slurry having a straw concentration of 50 wt % to 65 wt %.

The vegetable oil residue in the present invention selected from the group consisting of palm oil residue, soybean oil residue, peanut oil residue, saponin oil residue, linseed oil residue, castor oil residue, rapeseed oil residue, olive oil residue, and any combination thereof.

Said subjecting the vegetable oil residue to compression is carried out under a pressure of 3-5 MPa and a temperature of 40-60° C.

Said subjecting the vegetable oil residue to drying is carried out at a temperature of 80-110° C. for a period of 2-6 h to obtain a dried vegetable oil residue having a moisture content of less than 2 wt %, and after the first pulverization the dried vegetable oil residue has a median particle size of 100-300  $\mu\text{m}$ , and after the second pulverization the dried vegetable oil residue has a median particle size of 30-50  $\mu\text{m}$  and a bulk density of 1500-1600 kg/m<sup>3</sup>.

The slurry has a viscosity of 300-700 MPa·s (50° C.).

The grinding pulping is stirring pulping, dispersing pulping, emulsifying pulping, shearing pulping, or homogeneous pulping.

The vulcanizing agent can be sulfur, carbon disulfide or dimethyl disulfide.

The oils used in the preparation of the slurry, the types and amounts of the catalyst, the specific method of introducing hydrogen into the slurry, the introduction of cold hydrogen,

the amount of catalyst stored in the slurry bed reactor, the reaction time, and the method for preparing biomass charcoal loading with an active component, etc. are the same as those in the technical solution provided in the first aspect.

In a fourth aspect, the present invention also provides a fourth technical solution for one-pot liquefaction process for biomass, comprising: preparing a slurry containing a catalyst, a vulcanizing agent and a biomass, and introducing hydrogen into the slurry to carry out a reaction under a pressure of 15-20 MPa and a temperature of 300-400° C., obtaining a bio-oil.

The slurry is prepared with using straw as the biomass according to the following steps: subjecting the straw sequentially to drying, a first pulverization, compression and a second pulverization to obtain a pretreated biomass, and then mixing the pretreated biomass with the catalyst and the vulcanizing agent to obtain a mixture, and adding the mixture to an oil to carry out grinding pulping to obtain the slurry having a straw concentration of 35 to 50 wt %.

Said subjecting the straw to compression is carried out under a pressure of 2-5 MPa and a temperature of 30-60° C.

Said subjecting the straw to drying is carried out at a temperature of 70-110° C. for a period of 3-5 h to obtain a dried straw having a moisture content of less than 2 wt %, and after the first pulverization the dried straw has a median particle size of 100-300  $\mu\text{m}$ , and after the second pulverization the dried straw has a median particle size of 30-50  $\mu\text{m}$  and a bulk density of 400-800 kg/m<sup>3</sup>.

The slurry has a viscosity of 400-800 mPa·s (50° C.).

The grinding pulping is stirring pulping, dispersing pulping, emulsifying pulping, shearing pulping, or homogeneous pulping.

Said introducing hydrogen into the slurry comprises:

introducing a high-pressure hydrogen into the slurry to prepare a reaction raw material mixture, wherein the high-pressure hydrogen and the slurry have a volume ratio of (600-1500):1; and

heating the reaction raw material mixture to 300-400° C. and feeding it into a slurry bed reactor to undergo hydrolysis, cracking and hydrogenation reactions, and simultaneously introducing a cold hydrogen into the slurry bed reactor by controlling the slurry bed reactor to have a total gas velocity of 0.02-0.2 m/s, preferably 0.05-0.08 m/s;

wherein, the high-pressure hydrogen has a pressure of 15-22 MPa, and the cold hydrogen has a temperature of 60-135° C.

Said introducing the high-pressure hydrogen into the slurry comprises two steps of:

firstly, introducing a high-pressure hydrogen into the slurry till the volume ratio of the high-pressure hydrogen to the slurry is (50-200):1, and heating the slurry to 200-280° C., and

secondly, introducing a high-pressure hydrogen into the slurry.

The cold hydrogen is injected via 3-5 injection ports which are sequentially formed in a height direction in a side wall of the slurry bed reactor.

The catalyst stored in the slurry bed reactor is controlled in an amount of 5-30 wt % of the mass of liquid phase in the slurry bed reactor; and the reaction is carried out for 30-60 min.

The vulcanizing agent can be sulfur, carbon disulfide or dimethyl disulfide.

The types and amounts of the catalyst, and the method for preparing biomass charcoal loading with an active component, etc. are the same as those in the first technical solution of the present invention.

In a fifth aspect, the present invention also provides a fifth technical solution for one-pot liquefaction process for biomass, comprising the following steps:

preparing a slurry containing a catalyst, a vulcanizing agent and a biomass, and introducing hydrogen into the slurry to carry out a reaction under a pressure of 15-20 MPa and a temperature of 340-420° C., thereby obtaining a bio-oil;

wherein, the slurry is prepared with using a vegetable oil residue as the biomass according to the following steps: subjecting the vegetable oil residue sequentially to drying, a first pulverization, compression and a second pulverization to obtain a pretreated biomass, and then mixing the pretreated biomass with the catalyst and the vulcanizing agent to obtain a mixture, and adding the mixture to an oil to carry out grinding pulping to obtain the slurry having a vegetable oil residue concentration of 40 wt % to 50 wt %.

Said subjecting the straw to compression is carried out under a pressure of 0.5-3 MPa and a temperature of 30-50° C.

Said subjecting the vegetable oil residue to drying is carried out at a temperature of 80-110° C. for a period of 2-6 h to obtain a dried straw having a moisture content of less than 2 wt %, and after the first pulverization the dried straw has a median particle size of 50-300  $\mu\text{m}$ , and after the second pulverization the dried straw has a median particle size of 30-50  $\mu\text{m}$  and a bulk density of 1400-1600 kg/m<sup>3</sup>.

The slurry has a viscosity of 300-650 mPa·s (50° C.).

The grinding pulping is stirring pulping, dispersing pulping, emulsifying pulping, shearing pulping, or homogeneous pulping.

Said introducing hydrogen into the slurry comprises:

introducing a high-pressure hydrogen into the slurry to prepare a reaction raw material mixture, wherein the high-pressure hydrogen and the slurry have a volume ratio of (600-1500):1; and

heating the reaction raw material mixture to 340-420° C. and feeding it into a slurry bed reactor to undergo hydrolysis, cracking and hydrogenation reactions, and simultaneously introducing a cold hydrogen into the slurry bed reactor by controlling the slurry bed reactor to have a total gas velocity of 0.02-0.2 m/s, preferably 0.05-0.08 m/s;

wherein, the high-pressure hydrogen has a pressure of 15-22 MPa, and the cold hydrogen has a temperature of 60-135° C.

Said introducing the high-pressure hydrogen into the slurry comprises two steps of:

firstly, introducing a high-pressure hydrogen into the slurry till the volume ratio of the high-pressure hydrogen to the slurry is (50-200):1, and heating the slurry to 200-280° C., and secondly, introducing a high-pressure hydrogen into the slurry.

The catalyst stored in the slurry bed reactor is controlled in an amount of 5-30 wt % of the mass of liquid phase in the slurry bed reactor; and the reaction is carried out for 30-60 min.

The vulcanizing agent can be sulfur, carbon disulfide or dimethyl disulfide.

The types and amounts of the catalyst, the introduction of cold hydrogen, and the method for preparing biomass charcoal loading with an active component, etc. are the same as those in the first technical solution of the present invention.

In a sixth aspect, the present invention also provides a sixth technical solution for one-pot liquefaction process for biomass, comprising the following steps:

preparing a biomass coal slurry by mixing a biomass powder, a coal powder, a catalyst, and a vulcanizing agent

with an oil, and perform grinding pulping, wherein the biomass powder and the coal powder account for 60-70 wt % of the mass of the biomass coal slurry; and wherein the biomass powder is prepared by collecting a biomass and controlling the biomass to have a moisture content of less than 2 wt %, then pulverizing the biomass to a median particle size of 100-300  $\mu\text{m}$ , compressing and molding the pulverized biomass under a pressure of 2-5 MPa and a temperature of 30-60° C., and pulverizing the compressed biomass again to a median particle size of 30-50  $\mu\text{m}$ ; and wherein the coal powder is prepared by collecting a coal and controlling the coal to have a moisture content of less than 2 wt %, then pulverizing it to a median particle size of 50-100  $\mu\text{m}$  under a temperature of 30-60° C., compressing and molding the pulverized coal under a pressure of 5-15 MPa, and pulverizing the compressed coal again to a median particle size of 30-50  $\mu\text{m}$ ;

carrying out a liquefaction reaction, comprising introducing hydrogen into the biomass coal slurry to carry out a reaction under a pressure of 15 to 25 MPa and a temperature of 380-460° C. to finally obtain a bio-oil;

said preparing a biomass coal slurry comprises: firstly removing dust from the biomass powder and the coal powder, and premixing them with the catalyst and the vulcanizing agent to obtain a premix, and then mixing the premix with the oil; or directly mixing the biomass powder, the coal powder, and the catalyst with the oil.

The biomass accounts for 20-30 wt % of the mass of the biomass coal slurry, and the coal powder accounts for 30-45 wt % of the mass of the biomass coal slurry.

The moisture content is controlled by drying and dehydrating under a temperature of 50-70° C. for a period of 3-5 h.

The compression molding is a briquetting molding, a tabletting molding or a layering molding.

Said preparing a biomass coal slurry comprises controlling the biomass powder to have a bulk density of 300-500  $\text{kg/m}^3$ , and controlling the coal powder to have a bulk density of 1000-1200  $\text{kg/m}^3$ .

The pulverization is hammer mill pulverization, ball mill pulverization, rod mill pulverization, ultrafine pulverization or jet pulverization.

The grinding pulping is stirring pulping, dispersing pulping, emulsifying pulping, shearing pulping, homogeneous pulping and colloid grinder pulping.

The grinding pulping lasts for 2-8 min.

The biomass coal slurry has a viscosity of 550-1000  $\text{mPa}\cdot\text{s}$  (50° C.).

The coal is low rank coal. The oil is selected from the group consisting of hogwash oil, gutter oil, rancid oil, waste lubricating oil, waste engine oil, heavy oil, residual oil, washing oil, anthracene oil, coal tar, petroleum, bio-oil produced by the present process, and any combination thereof.

The catalyst is present in an amount of 1-10 wt %, preferably 1-4 wt %, of the total mass of the biomass and coal; and the catalyst has a particle size of 5-500  $\mu\text{m}$ .

Said introducing hydrogen is carried out by:

injecting high-pressure hydrogen into the slurry till the volume ratio of the high-pressure hydrogen to the slurry is (600-1500):1; thereby obtaining a reaction raw material mixture; and

heating the reaction raw material mixture to 320-450° C., feeding the heated reaction raw material mixture into a slurry bed reactor to undergo liquidation, cracking and hydrogenation reactions, and meanwhile, injecting cold hydrogen into the slurry bed reactor, wherein a total gas

speed in the slurry bed reactor is controlled within 0.02-0.2 m/s, preferably 0.05-0.08 m/s;

wherein, the high-pressure hydrogen has a pressure of 13-27 MPa, and the cold hydrogen has a temperature of 60-135° C.

Said injecting the high-pressure hydrogen into the slurry comprises two steps of:

injecting the high-pressure hydrogen into the slurry for the first time till the volume ratio of the high-pressure hydrogen to the slurry is (50-200):1, and

heating the slurry to 200-350° C., and injecting the high-pressure hydrogen into the slurry for the second time.

The cold hydrogen is injected via 3-5 injection ports which are sequentially formed in a height direction in a side wall of the slurry bed reactor.

The catalyst stored in the slurry bed reactor is controlled in an amount of 5-30 wt % of the mass of liquid in the slurry bed reactor; and the reaction is carried out for 30-90 min.

The biomass can be solid, such as straw of crops such as wheat, rice, corn, cotton, etc., or may be cash crops such as reeds, tabasheer grass, trees, leaves, fruits and vegetables, or algae, industrial wood, paper waste, etc.; the biomass may also be liquid, such as liquid stools; the biomass can be one biomass or a biomass raw material composed of a variety of biomass.

The types and composition of the catalyst, the types of vulcanizing agent, and the method for preparing biomass charcoal loading with a second active component are the same as those in the second technical solution of the present invention.

In a seventh aspect, the present invention also provides a seventh technical solution for one-pot liquefaction process for biomass, comprising the following steps:

preparing a biomass water coal slurry by mixing a biomass powder, a coal powder, a catalyst, and a vulcanizing agent with water, and perform grinding pulping, wherein, the biomass powder and the coal powder account for 55-65 wt % of the mass of the biomass water coal slurry; and wherein the biomass powder is prepared by collecting a biomass and controlling the biomass to have a moisture content of less than 2 wt %, then pulverizing the biomass to a median particle size of 100-300  $\mu\text{m}$ , compressing and molding the pulverized biomass under a pressure of 2-5 MPa and a temperature of 30-60° C., and pulverizing the compressed biomass again to a median particle size of 30-50  $\mu\text{m}$ ; and wherein the coal powder is prepared by collecting a coal and controlling the coal to have a moisture content of less than 2 wt %, then pulverizing it to a median particle size of 50-100  $\mu\text{m}$  under a temperature of 30-60° C., compressing and molding the pulverized coal under a pressure of 5-15 MPa, and pulverizing the compressed coal again to a median particle size of 30-100  $\mu\text{m}$ ;

carrying out a liquefaction reaction, comprising introducing hydrogen into the biomass water coal slurry to carry out a reaction under a pressure of 15 to 25 MPa and a temperature of 300 to 460° C. to finally obtain a bio-oil;

said preparing a biomass water coal slurry comprises: firstly removing dust from the biomass powder and the coal powder, and premixing them with the catalyst and the vulcanizing agent to obtain a premix, and then mixing the premix with water; or directly mixing the biomass powder, the coal powder, and the catalyst with water.

The biomass accounts for 15-30 wt % of the mass of the biomass water coal slurry, and the coal powder accounts for 35-50 wt % of the mass of the biomass water coal slurry.

## 11

The moisture content is controlled by drying and dehydrating under a temperature of 50-70° C. for a period of 3-5 h.

Said preparing a biomass water coal slurry comprises controlling the biomass powder to have a bulk density of 300-500 kg/m<sup>3</sup>, and controlling the coal powder to have a bulk density of 1200-1300 kg/m<sup>3</sup>.

The grinding pulping lasts for 2-8 min.

The coal is low rank coal.

In the biomass water coal slurry the catalyst is present in an amount of 1-10 wt %, preferably 1-4 wt %, of the total mass of the biomass and coal; and the catalyst has a particle size of 5-500 µm.

Wherein, the method for introducing hydrogen, the amount of the catalyst stored in the slurry bed reactor, the reaction time, the types and composition of the catalyst, the types of vulcanizing agent, the types of biomass, and the method for preparing biomass charcoal loading with a second active component are all the same as those in the sixth technical solution.

The technical solution of the present invention has the following advantages:

1. In the first one-pot liquefaction process for biomass provided by the present invention, the slurry is prepared with using straw as the biomass according to the following steps: subjecting the straw sequentially to drying, a first pulverization, compression and a second pulverization to obtain a pretreated biomass, and then mixing the pretreated biomass with the catalyst and the vulcanizing agent to obtain a mixture, and adding the mixture to an oil to carry out grinding pulping to obtain the slurry having a straw concentration of 30 wt % to 60 wt %. It is the first time to adopt a treatment process of subjecting the straw firstly to compression and then to a second pulverization. Through compression, loose straws undergo collapsing and closing, causing re-displacement and mechanical deformation, which results in reducing of volume of the straw, thereby reducing the porosity of the straw and increasing its density and specific gravity, so that the straws can be easily dispersed in oil, thus increasing its content in the oil and increasing the concentration of the reaction material. The straw is present in the slurry of the present invention in an amount of as high as 30-60 wt %, which is much higher than 5-16 wt % in the existing technology. Meanwhile, the increase of the straw concentration in the slurry will also increase the amount of biomass delivered by the pump per unit time, thereby increasing the efficiency of the entire biomass liquefaction process, reducing industrial costs and energy consumption. In addition, the increase in the specific gravity of the straw is also conducive to the suspension and dispersion of biomass in the slurry, thereby reducing the viscosity of the biomass slurry, achieving smooth flow of the slurry in the pipeline, avoiding clogging of the pipeline, achieving smooth operation and transportation of the pump, and also making it possible to use high viscosity waste oils such as waste engine oil, waste oil, and rancid oil that cannot be used as a biomass liquefied solvent in the prior art.

The second one-pot liquefaction process for biomass provided by the present invention comprises the following steps: preparing a slurry containing a catalyst, a vulcanizing agent and a biomass, and introducing hydrogen into the slurry to carry out a reaction under a pressure of 13-25 MPa and a temperature of 300-500° C., thereby obtaining a bio-oil. According to the process of the present invention, the biomass is subjected to a high-pressure high-temperature hydrolysis reaction in the presence of an appropriate amount of water (namely water inherently contained in the biomass),

## 12

and the resulted hydrolysis product further undergoes cracking and hydrogenation reactions under the action of hydrogenation and a catalyst, namely amorphous alumina loading oxides of metals of group VIB, group VIIIB or group VIII, thereby realizing conversion from the biomass to the bio-oil. In the process provided by the present invention, the conversion ratio of the biomass is up to 90-100%, the yield of the bio-oil is 60-86% or more, and the rate of coke formation is lower than 0.1%.

In the third one-pot liquefaction process for biomass provided by the present invention, the slurry is prepared as follows: subjecting the vegetable oil residue sequentially to drying, a first pulverization, compression and a second pulverization to obtain a pretreated biomass, and then mixing the pretreated biomass with the catalyst and the vulcanizing agent to obtain a mixture, and adding the mixture to an oil to carry out grinding pulping to obtain the slurry having a straw concentration of 50 wt % to 65 wt %. It is the first time to adopt a treatment process of subjecting the vegetable oil residue firstly to compression and then to a second pulverization. Through compression, loose vegetable oil residue undergoes collapsing and closing, causing re-displacement and mechanical deformation, which results in reducing of the volume of the vegetable oil residue, thereby reducing the porosity of the vegetable oil residue and increasing its density and specific gravity, making it easy to disperse in the oil and thus increasing its content in the oil, thereby increasing the concentration of the reaction material. The vegetable oil residue is present in the slurry of the present invention in an amount of as high as 50-65 wt %. Meanwhile, the increase of the vegetable oil residue concentration in the slurry will also increase the amount of biomass delivered by the pump per unit time, thereby increasing the efficiency of the entire biomass liquefaction process, reducing industrial costs and energy consumption. In addition, the increase in the specific gravity of the vegetable oil residue is also conducive to the suspension and dispersion of biomass in the slurry, thereby reducing the viscosity of the biomass slurry, achieving smooth flow of the slurry in the pipeline, avoiding clogging of the pipeline, achieving smooth operation and transportation of the pump, and also making it possible to use high viscosity waste oils such as waste engine oil, waste oil, and rancid oil that cannot be used as a biomass liquefied solvent in the prior art.

In the present invention, a slurry containing a catalyst, a vulcanizing agent and a biomass is prepared, and hydrogen is introduced into the slurry to carry out a reaction under a pressure of 15-25 MPa and a temperature of 380-480° C., thereby obtaining a bio-oil. According to the process of the present invention, the biomass undergoes cracking and hydrogenation reactions under the action of hydrogenation and a catalyst, thereby implementing conversion from the biomass to the bio-oil. In the process provided by the present invention, the conversion ratio of the biomass is up to 95-99%.

In the fourth one-pot liquefaction process for biomass provided by the present invention, the slurry is prepared with using straw as the biomass according to the following steps: subjecting the straw sequentially to drying, a first pulverization, compression and a second pulverization to obtain a pretreated biomass, and then mixing the pretreated biomass with the catalyst and the vulcanizing agent to obtain a mixture, and adding the mixture to water to carry out grinding pulping to obtain the slurry having a straw concentration of 35 wt % to 50 wt %. It is the first time to adopt a treatment process of subjecting the straw firstly to compression and then to a second pulverization. Through com-

pression, the loose straw undergoes collapsing and closing, causing re-displacement and mechanical deformation, which results in reducing of the volume of the straw, thereby reducing the porosity of the straw and increasing its density and specific gravity, making it easy to disperse in water and thus increasing its content in water, thereby increasing the concentration of the reaction material. Meanwhile, the increase of the straw concentration in the slurry will also increase the amount of biomass delivered by the pump per unit time, thereby increasing the efficiency of the entire biomass liquefaction process, reducing industrial costs and energy consumption. In addition, the increase in the specific gravity of the straw is also conducive to the suspension and dispersion of biomass in the slurry, thereby reducing the viscosity of the biomass slurry, achieving smooth flow of the slurry in the pipeline, avoiding clogging of the pipeline, achieving smooth operation and transportation of the pump.

In the present invention, a slurry containing a catalyst, a vulcanizing agent and a biomass is prepared, and hydrogen is introduced into the slurry to carry out a reaction under a pressure of 15-20 MPa and a temperature of 300-400° C., thereby obtaining a bio-oil. According to the process of the present invention, the biomass undergoes cracking and hydrogenation reactions under the action of hydrogenation and a catalyst, thereby implementing conversion from the biomass to the bio-oil, and improving the yield of the bio-oil. In the process provided by the present invention, the conversion ratio of the biomass is up to 95-99%, the yield of the bio-oil is 60-80%, and the residue in the bio-oil is less than 0.1 wt %.

In the fifth one-pot liquefaction process for biomass provided by the present invention, the slurry is prepared as follows: subjecting the vegetable oil residue sequentially to drying, a first pulverization, compression and a second pulverization to obtain a pretreated biomass, and then mixing the pretreated biomass with the catalyst and the vulcanizing agent to obtain a mixture, and adding the mixture to water to carry out grinding pulping to obtain the slurry having a straw concentration of 40 wt % to 50 wt %. It is the first time in the present invention to adopt a treatment process of subjecting the vegetable oil residue firstly to compression and then to a second pulverization. Through compression, the loose vegetable oil residue undergoes collapsing and closing, causing re-displacement and mechanical deformation, which results in reducing of volume of the vegetable oil residue, thereby reducing the porosity of the vegetable oil residue and increasing its density and specific gravity, making it easy to disperse in the water and thus increasing its content in water, thereby increasing the concentration of the reaction material. Meanwhile, the increase of the vegetable oil residue concentration in the slurry will also increase the amount of biomass delivered by the pump per unit time, thereby increasing the efficiency of the entire biomass liquefaction process, reducing industrial costs and energy consumption. In addition, the increase in the specific gravity of the vegetable oil residue is also conducive to the suspension and dispersion of biomass in the slurry, thereby reducing the viscosity of the biomass slurry, achieving smooth flow of the slurry in the pipeline, avoiding clogging of the pipeline, achieving smooth operation and transportation of the pump.

In the present invention, the slurry containing a catalyst, a vulcanizing agent and a biomass is prepared, and hydrogen is introduced into the slurry to carry out a reaction under a pressure of 15-20 MPa and a temperature of 340-420° C. According to the process of the present invention, the biomass undergoes cracking and hydrogenation reactions

under the action of hydrogenation and a catalyst, thereby implementing conversion from the biomass to the bio-oil. In the process provided by the present invention, the conversion ratio of the biomass is up to 95-99%, the yield of the bio-oil is 70-86%, and the residue in the bio-oil is less than 0.1 wt %.

In the seventh one-pot liquefaction process for biomass provided by the present invention, it is the first time to realize co-liquefaction of coal and biomass with water as a hydrogen-donor solvent. The present invention successfully prepares a biomass coal water slurry having a biomass and coal content of 55-65 wt %, and a viscosity of only 450-1100 mPa·s (50° C.) by a process of subjecting the biomass and coal to dehydrating, pulverizing, compressing, re-pulverizing, a first pulping, and grinding, and by optimizing the pulverized particle size and compression conditions.

2. In the first one-pot liquefaction process provided by the present invention, the compression temperature is controlled at 30-60° C. Compressing the straw at this temperature can significantly enhance the rheological properties of the straw and reduce the viscosity of the biomass slurry. The slurry formed by straw and oil in the process of the present invention has a viscosity of 500-1400 mPa·s (50° C.), thereby achieving smooth flow of the slurry in the pipeline, avoiding clogging of the pipeline, achieving smooth operation and transportation of the pump.

In the third one-pot liquefaction process provided by the present invention, the compression temperature is controlled at 40-60° C. Compressing the vegetable oil residue at this temperature can significantly enhance the rheological properties of the vegetable oil residue and reduce the viscosity of the biomass slurry. The slurry formed by the vegetable oil residue and oil in the process of the present invention has a viscosity of 300-700 mPa·s (50° C.), thereby achieving smooth flow of the slurry in the pipeline, avoiding clogging of the pipeline, achieving smooth operation and transportation of the pump.

In the fourth one-pot liquefaction process provided by the present invention, the compression temperature is controlled at 30-60° C. Compressing the straw at this temperature can significantly enhance the rheological properties of the straw and reduce the viscosity of the biomass slurry. The slurry formed by straw and oil in the process of the present invention has a viscosity of 400-800 mPa·s (50° C.), thereby achieving smooth flow of the slurry in the pipeline, avoiding clogging of the pipeline, achieving smooth operation and transportation of the pump.

In the fifth one-pot liquefaction process provided by the present invention, the compression temperature is controlled at 30-50° C. Compressing the vegetable oil residue at this temperature can significantly enhance the rheological properties of the vegetable oil residue and reduce the viscosity of the biomass slurry. The slurry formed by the vegetable oil residue and oil in the process of the present invention has a viscosity of 300-650 mPa·s (50° C.), thereby achieving smooth flow of the slurry in the pipeline, avoiding clogging of the pipeline, achieving smooth operation and transportation of the pump.

In the sixth technical solution of the present invention, it is the first time to realize co-liquefaction of coal, biomass and oil. The present invention successfully prepares a biomass coal slurry having a biomass and coal content of 60-70 wt %, and a viscosity of only 550-1000 mPa·s (50° C.) by a process of subjecting the biomass and coal to dehydrating, pulverizing, compressing, re-pulverizing, a first pulping, and grinding, and by optimizing the pulverized particle size and compression conditions.

In the seventh one-pot liquefaction process for biomass provided by the present invention, it is the first time to realize co-liquefaction of coal and biomass with water as a hydrogen-donor solvent. The present invention successfully prepares a biomass coal water slurry having a biomass and coal content of 55-65 wt %, and a viscosity of only 450-1100 mPa·s (50° C.) by a process of subjecting the biomass and coal to dehydrating, pulverizing, compressing, re-pulverizing, a first pulping, and grinding, and by optimizing the pulverized particle size and compression conditions.

In the one-pot liquefaction process for biomass provided by the present invention, compression can cause the pore structure inside the coal and biomass material to collapse and close, resulting in plastic flow and plastic deformation, thereby greatly increasing the density of the coal and biomass raw materials, so that they can be well dispersed in the solvent oil. Meanwhile, the collapse and closure of the pore structure prevents the coal and biomass from absorbing the solvent oil, so that the solvent oil can fully play its role as a dispersant. The inventors have found that the compression temperature has a great influence on the degree of plastic rheology and plastic deformation. The higher the temperature is, the greater the density becomes. However, excessive temperature will cause the material to decompose or cause other problems. Therefore, a temperature of 30° C. to 60° C. is adopted for the compression. The re-pulverization operation after compression increases the contactable area of the raw material, so that the raw material can be in better contact with the catalyst and the solvent oil, thus enhancing the transfer of hydrogen, greatly reducing situations that the raw material cannot contact with hydrogen and catalyst due to being in a porous structure.

The process of “a first pulverization+compression+a second pulverization” provided by the present invention can be applied to all coal materials and biomass materials having pore structure, especially low-rank coal materials such as lignite, and porous biomass materials such as straw and rice husk. The resulting high-concentration biomass coal slurry has good slurryability and high fluidity, and can be directly transported smoothly by the pump, which not only effectively improve the operation stability of the delivery system, the utilization efficiency of the liquefaction device and the liquefaction efficiency, satisfying the feeding requirements of the subsequent treatment process, but also realizes clean and efficient use of inferior coal and biomass. The close proximity between the coal and the biomass enables the hydrogen produced by biomass pyrolysis to be used as part of hydrogen source for coal pyrolysis, reducing the hydrogen consumption. Through the co-liquefaction process provided by the present invention, high-viscosity waste oils, such as waste engine oil, gutter oil and rancidity oil, which cannot be used as the liquefaction solvent of the coal and the biomass in the existing technology, can also be utilized.

In the sixth technical solution provided by the present invention, bio-oil is obtained by introducing hydrogen into the slurry to carry out a reaction under a pressure of 13-25 MPa and a temperature of 300-500° C. The process of the present invention enables the coal and the biomass to undergo liquefaction at high-pressure and high-temperature, and the liquefaction product further undergoes cracking and hydrogenation reactions under the action of hydrogenation and a catalyst, namely amorphous alumina loading oxides of metals of group VIB, group VIIB or group VIII, thereby implementing conversion from the biomass to the bio-oil. In the process provided by the present invention, the conver-

sion ratio of the biomass is up to 90-99%, the yield of the bio-oil is 60-80% or more, and amount of residue is no higher than 2.5 wt %.

In the seventh technical solution provided by the present invention, a bio-oil is obtained by introducing hydrogen into the slurry to carry out a reaction under a pressure of 15-25 MPa and a temperature of 300-460° C. According to the process of the present invention, the biomass is subjected to a high-pressure high-temperature hydrolysis reaction in the presence of an appropriate amount of water (namely water inherently contained in the biomass and coal), and the hydrolysis product further undergoes cracking and hydrogenation reactions under the action of hydrogenation and a catalyst, namely amorphous alumina loading oxides of metals of group VIB, group VIIB or group VIII, thereby implementing conversion from the biomass to the bio-oil. In the process provided by the present invention, the conversion ratio of the coal and the biomass is up to 90-95%, the yield of the bio-oil is 70-85% or more, and the rate of coke formation is lower than 5%.

The present invention can ensure the solid particles used for preparing the biomass oil coal slurry have uniform particle size by further cooperating with the screening process of the solid material, so that the obtained biomass coal slurry has better stability, and is difficult to settle during transportation, avoiding blockage of the transportation pipeline and damage to the liquefaction equipment.

In the present invention, the catalyst is preferably an amorphous alumina loading oxides of metals of group VIB, group VIIB or group VIII, or a composite catalyst of biomass charcoal and amorphous iron oxide. These catalysts have better hydrogenation performance after vulcanization with noble metal, and can prevent coke forming. The biomass charcoal or the amorphous alumina has acidity and cracking function, and the amorphous iron oxide has alkalinity, can facilitate liquefaction, and also has catalytic hydrogenation function after iron is vulcanized, thereby reducing consumption of the noble metal.

In the one-pot liquefaction process for coal and biomass provided by the present invention, coal and biomass are firstly subjected to pretreatment, such as drying, compression, crushing, dust-removing, etc., then mixed with the catalyst. In this way, the surface of coal and biomass powder can be greatly utilized and help the catalyst to attach to the surface of the solid powder, so that the catalyst can timely provide hydrogen transfer for the coal and biomass liquefaction product; therefore, ensuring no coke polycondensation occurs in the whole procedure of the one-pot liquefaction process, and a purpose of reducing residue is achieved.

3. In the one-pot liquefaction process for coal and biomass provided by the present invention, the catalyst is preferably selected from the group consisting of amorphous iron oxy-hydroxide, amorphous alumina loading with an active component, biomass charcoal loading an active component and any combination thereof, wherein the active component is selected from the group consisting of oxides of metals of group VIB, group VIIB, group VIII and any combination thereof in the periodic table of elements. Amorphous FeOOH is alkaline and can promote the hydrolysis. Biomass charcoal and amorphous alumina are inherently acidic, and have a function of pyrolysis, which can be enhanced when loading active components, thus avoiding the generation of coke in the process of biomass liquefaction.

4. In the one-pot liquefaction process for coal and biomass provided by the present invention, slurry bed reactor is adopted, into which the reaction raw material mixture is fed via the bottom thereof to carry out reaction. Meanwhile, cold

hydrogen is injected into the reactor, so that flow rate difference control of each phase state is implemented in the reactor depending on different specific weights of gas, liquid and solid materials and by matching with specific weight difference variation caused by the yield of a reacted light oil product. The biomass raw material mixture undergoes hydrolysis, cracking and hydrogenation reactions in the reactor from bottom to top; in such procedures, even though the biomass with a large specific weight and the catalyst solid particles with a large specific weight ascend along with the gas and the light oil product, the ascended biomass and catalyst solid particles return to the bottom of the reactor under the action of the upper-part cold hydrogen to undergo the reactions again, and the content of the hydrogen in the slurry and the injection amount of the cold hydrogen in the reactor are suitably adjusted according to the densities of materials in the upper part, middle part and lower part of the reactor, thereby implementing circulation of an unconverted biomass in the reactor and balance discharge of the catalyst; therefore, the reactions of hydrolysis, cracking, hydrogenation and the like are guaranteed to be carried out completely, which facilitates improvement on the conversion ratio of the biomass and the yield of an oil phase.

5. In the one-pot liquefaction process for coal and biomass provided by the present invention, the high-pressure hydrogen is injected into the slurry in the two steps, that is, the high-pressure hydrogen is injected once before and after the slurry is heated, respectively, and the former injection of the high-pressure hydrogen can improve perturbation of the slurry in a heat exchanger, thereby avoiding deposition of the solid biomass and the catalyst.

6. In the one-pot liquefaction process for coal and biomass provided by the present invention, the catalyst is preferably an amorphous alumina loading oxides of metals of group VIB, group VIIIB or group VIII, or a composite catalyst of biomass charcoal and amorphous iron oxide. These catalysts have better hydrogenation performance after vulcanized with noble metal and can prevent coke forming. The biomass charcoal or amorphous alumina have acidity and cracking function, and the amorphous iron oxide has alkalinity, can facilitate biomass hydrolysis, and also has catalytic hydrogenation function after iron is vulcanized, thereby reducing consumption of the noble metal.

7. In the one-pot liquefaction process for coal and biomass provided by the present invention, when the biomass raw material is solid, the solid biomass needs to be pretreated firstly, such as by drying, crushing, dust-removing, etc., to obtain a pretreated solid biomass, and then the pretreated solid biomass is mixed with the catalyst so as to greatly utilize the surface of biomass powder and help the catalyst to attach to the surface of the solid biomass powder, so that the catalyst can timely provide hydrogen transfer for the biomass hydrolysis product; therefore, it is ensured that no coke polycondensation occurs in the whole procedure of the one-pot liquefaction process for biomass, and a purpose of reducing the rate of coke formation is achieved.

#### DETAILED DESCRIPTION OF EMBODIMENTS

The technical solution of the present invention is described below clearly and completely. Apparently, the embodiments described below are a part, but not all, of the embodiments of the present invention. All other embodiments, obtained by those of ordinary skill in the art based on the embodiments of the present invention without any creative efforts, fall into the protection scope of the present invention. In addition, technical features involved in various

implementations of the present invention described below can be combined with each other as long as they do not conflict with each other.

#### 5 Embodiment 1

Provided is one-pot liquefaction process for biomass described as below.

##### 10 Pretreatment of Biomass:

Wheat straw and corn straw are fed into a drier for drying under a temperature of 50° C. for 5 h to have a moisture content of less than 2 wt %, and then fed to an ultrafine pulverizer for a first pulverization to a median particle size of 100 µm, then fed into a plodder for compressing at a temperature of 30° C. and a pressure of 3 MPa, and then extruded and molded, and then subjected to a second pulverization to produce a pretreated biomass having a median particle size of 30 µm and a bulk density of 500 kg/m<sup>3</sup>.

##### 20 Preparation of Catalyst:

S1, carrying out acidification on biomass charcoal to produce a biomass charcoal support; and

S2, subjecting Mo oxide and the above biomass charcoal support to vibration grinding to obtain a biomass charcoal loading Mo oxide having a particle size of 400-500 µm, i.e. a catalyst.

In the above catalyst, Mo accounts for 1% by weight of the above biomass charcoal support. The acidification is carried out with an acid medium which has H<sup>+</sup> concentration of 5 mol/L. A volume ratio of the carbonized biomass charcoal to the acid medium is 1:5, and the acidification is carried out at a temperature of 80° C. for a period of 1 h.

##### 35 Preparation of Biomass Slurry:

The pretreated biomass and the above catalyst are mixed with sulfur to obtain a mixture, and the mixture is added to a mixed oil of hogwash oil and residual oil to carry out stirring grinding to form a slurry. The wheat straw and corn straw are present in a total amount of 60 wt % in the slurry, and the slurry has a viscosity of 500 mPa·s (50° C.). Further, in the slurry, the catalyst accounts for 1 wt %, and the vulcanizing agent accounts for 0.4 wt % of the pretreated biomass.

##### 40 Liquefaction:

Introducing hydrogen into the slurry to carry out a reaction under a pressure of 25 MPa and a temperature of 380° C. to obtain a bio-oil.

Said introducing hydrogen into the slurry comprises: introducing a high-pressure hydrogen into the slurry to prepare a reaction raw material mixture, wherein the high-pressure hydrogen and the slurry have a volume ratio of 1500:1; and heating the reaction raw material mixture to 380° C. and feeding it into a slurry bed reactor to undergo hydrolysis, cracking and hydrogenation reactions, and simultaneously introducing a cold hydrogen into the slurry bed reactor by controlling the slurry bed reactor to have a total gas velocity of 0.2 m/s; wherein, the high-pressure hydrogen has a pressure of 27 MPa, and the cold hydrogen has a temperature of 135° C.

The cold hydrogen is injected via 3 injection ports which are sequentially formed in a height direction in a side wall of the slurry bed reactor. The biomass charcoal loading Mo oxide as a catalyst is stored in the slurry bed reactor in an amount of 30 wt % of the mass of liquid in the slurry bed reactor; and the reaction is carried out for a period of 30 min.

Provided is one-pot liquefaction process for biomass described as below.

Pretreatment of Biomass:

Palm oil residue is fed into a drier for drying under a temperature of 80° C. for 5 h to have a moisture content of less than 2 wt %, and then fed to an ultrafine pulverizer for a first pulverization to a median particle size of 100 µm, then fed into a briquetting press for compressing at a temperature of 50° C. and a pressure of 5 MPa, and then extruded and molded, and then subjected to a second pulverization to produce a pretreated biomass having a median particle size of 30 µm and a bulk density of 1600 kg/m<sup>3</sup>.

Preparation of Catalyst:

S1, carrying out acidification on biomass charcoal to produce a biomass charcoal support; and.

S2, subjecting Mo oxide and the above biomass charcoal support to vibration grinding to obtain a biomass charcoal loading Mo oxide having a particle size of 400-500 µm, i.e. a catalyst.

In the above catalyst, Mo accounts for 1% by weight of the above biomass charcoal support. The acidification is carried out with an acid medium which has a H<sup>+</sup> concentration of 5 mol/L. A volume ratio of the carbonized biomass charcoal to the acid medium is 1:5, and the acidification is carried out at a temperature of 80° C. for a period of 1 h.

Preparation of Biomass Slurry:

The pretreated biomass and the above catalyst are mixed with sulfur to obtain a mixture, and the mixture is added to a mixed oil of hogwash oil and residual oil to carry out stirring grinding to form a slurry. The palm oil residue is present in a total amount of 60 wt % in the slurry, and the slurry has a viscosity of 300 mPa·s (50° C.). Further, in the slurry, the catalyst accounts for 1 wt %, and the vulcanizing agent accounts for 0.4 wt % of the pretreated biomass.

Liquefaction:

Introducing hydrogen into the slurry to carry out a reaction under a pressure of 25 MPa and a temperature of 380° C. to obtain a bio-oil.

Said introducing hydrogen into the slurry comprises: introducing a high-pressure hydrogen into the slurry to prepare a reaction raw material mixture, wherein the high-pressure hydrogen and the slurry have a volume ratio of 1500:1; and heating the reaction raw material mixture to 380° C. and feeding it into a slurry bed reactor to undergo hydrolysis, cracking and hydrogenation reactions, and simultaneously introducing a cold hydrogen into the slurry bed reactor by controlling the slurry bed reactor to have a total gas velocity of 0.2 m/s; wherein, the high-pressure hydrogen has a pressure of 27 MPa, and the cold hydrogen has a temperature of 135° C.

The cold hydrogen is injected via 3 injection ports which are sequentially formed in a height direction in a side wall of the slurry bed reactor. The biomass charcoal loading Mo oxide as a catalyst is stored in the slurry bed reactor in an amount of 30 wt % of the mass of liquid in the slurry bed reactor; and the reaction is carried out for a period of 100 min.

Provided is one-pot liquefaction process for biomass described as below.

Pretreatment of Biomass:

Cotton straw is fed into a drier for drying under a temperature of 60° C. for 4 h to have a moisture content of

less than 2 wt %, and then fed to an ultrafine pulverizer for a first pulverization to a median particle size of 210 µm, then fed into a briquetting press for compressing at a temperature of 55° C. and a pressure of 2.1 MPa, and then extruded and molded, and then subjected to a second pulverization to produce a pretreated biomass having a median particle size of 40 µm and a bulk density of 440 kg/m<sup>3</sup>.

Preparation of Biomass Charcoal Loading Mo Oxide and Pd Oxide:

S1, carrying out acidification on biomass charcoal to produce a biomass charcoal support; and

S2, subjecting Mo oxide, Pd oxide and the above biomass charcoal support to vibration grinding to obtain a biomass charcoal loading Mo oxide and Pd oxide, having a particle size of 120-400 µm.

In the above biomass charcoal loading Mo oxide and Pd oxide, Mo and Pd account for 3.5% by weight of the above biomass charcoal support. The acidification is carried out with an acid medium which has a H<sup>+</sup> concentration of 3.5 mol/L. A volume ratio of the carbonized biomass charcoal to the acid medium is 1:10, and the acidification is carried out at a temperature of 50° C. for a period of 4.3 h.

Preparation of Biomass Slurry:

The pretreated biomass and the above biomass charcoal loading Mo oxide and Pd oxide are mixed with amorphous FeOOH and sulfur to obtain a mixture, and the mixture is added to a mixed oil of heavy oil and wash oil to carry out emulsifying pulping to form a slurry. The cotton straw are present in a total amount of 30 wt % in the slurry, and the slurry has a viscosity of 725 mPa·s (50° C.). Further, in the slurry, the biomass charcoal loading Mo oxide and Pd oxide and amorphous FeOOH (having a particle size of 150-200 µm) account for 6 wt %, and the vulcanizing agent accounts for 0.2 wt % of the pretreated biomass.

Liquefaction:

Introducing hydrogen into the slurry to carry out a reaction under a pressure of 20 MPa and a temperature of 400° C. to obtain a bio-oil.

Said introducing hydrogen into the slurry comprises: introducing a high-pressure hydrogen into the slurry to prepare a reaction raw material mixture, wherein the high-pressure hydrogen and the slurry have a volume ratio of 1000:1; and heating the reaction raw material mixture to 400° C. and feeding it into a slurry bed reactor to undergo hydrolysis, cracking and hydrogenation reactions, and simultaneously introducing a cold hydrogen into the slurry bed reactor by controlling the slurry bed reactor to have a total gas velocity of 0.10 m/s; wherein, the high-pressure hydrogen has a pressure of 21 MPa, and the cold hydrogen has a temperature of 80° C.

The cold hydrogen is injected via 4 injection ports which are sequentially formed in a height direction in a side wall of the slurry bed reactor. The biomass charcoal loading Mo oxide and Pd oxide as a catalyst is stored in the slurry bed reactor in an amount of 25 wt % of the mass of liquid in the slurry bed reactor; and the reaction is carried out for a period of 50 min.

Provided is one-pot liquefaction process for biomass described as below.

Pretreatment of Biomass:

Wheat straw and flax straw are fed into a drier for drying under a temperature of 65° C. for 4.5 h to have a moisture content of less than 2 wt %, and then fed to an ultrafine pulverizer for a first pulverization to a median particle size

of 180  $\mu\text{m}$ , then fed into a briquetting press for compressing at a temperature of 45° C. and a pressure of 2.6 MPa, and then extruded and molded, and then subjected to a second pulverization to produce a pretreated biomass having a median particle size of 36  $\mu\text{m}$  and a bulk density of 440 kg/m<sup>3</sup>.

Preparation of Biomass Slurry:

The pretreated biomass is mixed with amorphous FeOOH (having a particle size of 100-200  $\mu\text{m}$ ) and dimethyl disulfide to obtain a mixture, and the mixture is added to sour oil to carry out shearing pulping to form a slurry. The wheat straw and flax straw are present in a total amount of 55 wt % in the slurry, and the slurry has a viscosity of 620 mPa·s (50° C.). Further, in the slurry, amorphous FeOOH accounts for 6 wt % and the vulcanizing agent accounts for 0.25 wt % of the mass of the pretreated biomass.

Liquefaction:

Introducing hydrogen into the slurry to carry out a reaction under a pressure of 17 MPa and a temperature of 440° C. to obtain a bio-oil.

Said introducing the high-pressure hydrogen into the slurry comprises two steps of: firstly, introducing a high-pressure hydrogen into the slurry till the volume ratio of the high-pressure hydrogen to the slurry is 50:1, and heating the slurry to 200° C., and secondly, introducing a high-pressure hydrogen into the slurry, wherein the total volume of the high-pressure hydrogen introduced twice and the slurry have a volume ratio of 1300:1; and heating the reaction raw material mixture to 440° C. and feeding it into a slurry bed reactor to undergo hydrolysis, cracking and hydrogenation reactions, and simultaneously introducing a cold hydrogen into the slurry bed reactor by controlling the slurry bed reactor to have a total gas velocity of 0.05 m/s; wherein, the high-pressure hydrogen has a pressure of 16 MPa, and the cold hydrogen has a temperature of 105° C.

The cold hydrogen is injected via 4 injection ports which are sequentially formed in a height direction in a side wall of the slurry bed reactor. The amorphous FeOOH used as a catalyst is stored in the slurry bed reactor in an amount of 9 wt % of the mass of liquid in the slurry bed reactor; and the reaction is carried out for a period of 110 min.

Embodiment 5

Provided is one-pot liquefaction process for biomass described as below.

Pretreatment of Biomass:

Olive oil residue is fed into a drier for drying under a temperature of 90° C. for 3 h to have a moisture content of less than 2 wt %, and then fed to an ultrafine pulverizer for a first pulverization to a median particle size of 180  $\mu\text{m}$ , then fed into a briquetting press for compressing at a temperature of 60° C. and a pressure of 3.5 MPa, and then extruded and molded, and then subjected to a second pulverization to produce a pretreated biomass having a median particle size of 36  $\mu\text{m}$  and a bulk density of 1522 kg/m<sup>3</sup>.

Preparation of Biomass Slurry:

The pretreated biomass is mixed with amorphous FeOOH (having a particle size of 100-200  $\mu\text{m}$ ) and dimethyl disulfide to obtain a mixture, and the mixture is added to sour oil to carry out shearing pulping to form a slurry. The olive oil residue is present in a total amount of 55 wt % in the slurry, and the slurry has a viscosity of 617 mPa·s (50° C.). Further, in the slurry, amorphous FeOOH accounts for 6 wt % and the vulcanizing agent accounts for 0.25 wt % of the mass of the pretreated biomass.

Liquefaction:

Introducing hydrogen into the slurry to carry out a reaction under a pressure of 17 MPa and a temperature of 440° C. to obtain a bio-oil.

Said introducing the high-pressure hydrogen into the slurry comprises two steps of: firstly, introducing a high-pressure hydrogen into the slurry till the volume ratio of the high-pressure hydrogen to the slurry is 50:1, and heating the slurry to 200° C., and secondly, introducing a high-pressure hydrogen into the slurry, wherein the total volume of the high-pressure hydrogen introduced twice and the slurry have a volume ratio of 1300:1; and heating the reaction raw material mixture to 440° C. and feeding it into a slurry bed reactor to undergo hydrolysis, cracking and hydrogenation reactions, and simultaneously introducing a cold hydrogen into the slurry bed reactor by controlling the slurry bed reactor to have a total gas velocity of 0.05 m/s; wherein, the high-pressure hydrogen has a pressure of 16 MPa, and the cold hydrogen has a temperature of 105° C.

The cold hydrogen is injected via 4 injection ports which are sequentially formed in a height direction in a side wall of the slurry bed reactor. The amorphous FeOOH used as a catalyst is stored in the slurry bed reactor in an amount of 9 wt % of the mass of liquid in the slurry bed reactor; and the reaction is carried out for a period of 110 min.

Embodiment 6

Provided is one-pot liquefaction process for biomass described as below.

Pretreatment of Biomass:

Rapeseed oil residue is fed into a drier for drying under a temperature of 80° C. for 2 h to have a moisture content of less than 2 wt %, and then fed to an ultrafine pulverizer for a first pulverization to a median particle size of 200  $\mu\text{m}$ , then fed into a briquetting press for compressing at a temperature of 40° C. and a pressure of 3 MPa, and then extruded and molded, and then subjected to a second pulverization to produce a pretreated biomass having a median particle size of 45  $\mu\text{m}$  and a bulk density of 1600 kg/m<sup>3</sup>.

Preparation of Catalyst:

S1, carrying out alkalinization on biomass charcoal to produce a biomass charcoal support; and

S2, subjecting Ni oxide and the above biomass charcoal support to flat grinding and ball-milling to obtain a biomass charcoal loading Ni oxide having a particle size of 200-400  $\mu\text{m}$ , i.e. a catalyst.

In the above catalyst, Ni accounts for 1% by weight of the above biomass charcoal support. The alkalinization is carried out with an acid medium which has an OH<sup>+</sup> concentration of 0.5 mol/L. A volume ratio of the carbonized biomass charcoal to the alkaline medium is 1:15, and the alkalinization is carried out at a temperature of 30° C. for a period of 10 h.

Preparation of Biomass Slurry:

The pretreated biomass and the above catalyst are mixed with carbon disulfide to obtain a mixture, and the mixture is added to sour oil to carry out shearing pulping to form a slurry. The Rapeseed oil residue is present in a total amount of 59 wt % in the slurry, and the slurry has a viscosity of 305 mPa·s (50° C.). Further, in the slurry, the catalyst accounts for 1 wt % and the vulcanizing agent accounts for 0.25 wt % of the mass of the pretreated biomass.

Liquefaction:

Introducing hydrogen into the slurry to carry out a reaction under a pressure of 15 MPa and a temperature of 380° C. to obtain a bio-oil.

Said introducing hydrogen into the slurry comprises: introducing a high-pressure hydrogen into the slurry to

prepare a reaction raw material mixture, wherein the high-pressure hydrogen and the slurry have a volume ratio of 600:1; and heating the reaction raw material mixture to 380° C. and feeding it into a slurry bed reactor to undergo hydrolysis, cracking and hydrogenation reactions, and simultaneously introducing a cold hydrogen into the slurry bed reactor by controlling the slurry bed reactor to have a total gas velocity of 0.2 m/s; wherein, the high-pressure hydrogen has a pressure of 18 MPa, and the cold hydrogen has a temperature of 135° C.

The cold hydrogen is injected via 5 injection ports which are sequentially formed in a height direction in a side wall of the slurry bed reactor. The biomass charcoal loading Ni oxide as a catalyst is stored in the slurry bed reactor in an amount of 30 wt % of the mass of liquid in the slurry bed reactor; and the reaction is carried out for a period of 90 min.

#### Embodiment 7

Provided is one-pot liquefaction process for biomass described as below.

##### Pretreatment of Biomass:

Rice straw and reed straw are fed into a drier for drying under a temperature of 70° C. for 5 h to have a moisture content of less than 2 wt %, and then fed to an ultrafine pulverizer for a first pulverization to a median particle size of 100 µm, then fed into a briquetting press for compressing at a temperature of 60° C. and a pressure of 2 MPa, and then extruded and molded, and then subjected to a second pulverization to produce a pretreated biomass having a median particle size of 30 µm and a bulk density of 400 kg/m<sup>3</sup>.

##### Preparation of Catalyst:

S1, carrying out acidification on biomass charcoal to produce a biomass charcoal support; and.

S2, subjecting Mo oxide and the above biomass charcoal support to vibration grinding to obtain a biomass charcoal loading Mo oxide having a particle size of 400-500 m, i.e. a catalyst.

In the above catalyst, Mo accounts for 1% of the mass of the above biomass charcoal support. The acidification is carried out with an acid medium which has a H<sup>+</sup> concentration of 5 mol/L. A volume ratio of the carbonized biomass charcoal to the acid medium is 1:5, and the acidification is carried out at a temperature of 80° C. for a period of 1 h.

##### Preparation of Biomass Slurry:

The pretreated biomass and the above catalyst are mixed with sulfur to obtain a mixture, and the mixture is added to water to carry out stirring grinding to form a slurry. The rice straw and reed straw are present in a total amount of 50 wt % in the slurry, and the slurry has a viscosity of 800 mPa·s (50° C.). Further, in the slurry, the catalyst accounts for 1 wt % and the vulcanizing agent accounts for 0.4 wt % of the mass of the pretreated biomass.

##### Liquefaction:

Introducing hydrogen into the slurry to carry out a reaction under a pressure of 20 MPa and a temperature of 300° C. to obtain a bio-oil.

Said introducing hydrogen into the slurry comprises: introducing a high-pressure hydrogen into the slurry to prepare a reaction raw material mixture, wherein the high-pressure hydrogen and the slurry have a volume ratio of 1500:1; and heating the reaction raw material mixture to 320° C. and feeding it into a slurry bed reactor to undergo hydrolysis, cracking and hydrogenation reactions, and simultaneously introducing a cold hydrogen into the slurry bed reactor by controlling the slurry bed reactor to have a

total gas velocity of 0.2 m/s; wherein, the high-pressure hydrogen has a pressure of 22 MPa, and the cold hydrogen has a temperature of 135° C.

The cold hydrogen is injected via 3 injection ports which are sequentially formed in a height direction in a side wall of the slurry bed reactor. The biomass charcoal loading Mo oxide as a catalyst is stored in the slurry bed reactor in an amount of 30 wt % of the mass of liquid in the slurry bed reactor; and the reaction is carried out for a period of 30 min.

#### Embodiment 8

Provided is one-pot liquefaction process for biomass described as below.

##### Pretreatment of Biomass:

Olive oil residue is fed into a drier for drying under a temperature of 100° C. for 4.0 h to have a moisture content of less than 2 wt %, and then fed to an ultrafine pulverizer for a first pulverization to a median particle size of 290 µm, then fed into a briquetting press for compressing at a temperature of 35° C. and a pressure of 2.7 MPa, and then extruded and molded, and then subjected to a second pulverization to produce a pretreated biomass having a median particle size of 44 µm and a bulk density of 1510 kg/m<sup>3</sup>.

##### Preparation of Biomass Slurry:

The pretreated biomass is mixed with amorphous FeOOH (having a particle size of 100-200 µm) and sulfur to obtain a mixture, and the mixture is added to water to carry out shearing grinding to form a slurry. The olive oil residue is present in a total amount of 50 wt % in the slurry, and the slurry has a viscosity of 465 mPa·s (50° C.). Further, in the slurry, amorphous FeOOH accounts for 6 wt % and the vulcanizing agent accounts for 0.25 wt % of the mass of the pretreated biomass.

##### Liquefaction:

Introducing hydrogen into the slurry to carry out a reaction under a pressure of 18 MPa and a temperature of 340° C. to obtain a bio-oil.

Said introducing the high-pressure hydrogen into the slurry comprises two steps of: firstly, introducing a high-pressure hydrogen into the slurry till the volume ratio of the high-pressure hydrogen to the slurry is 50:1, and heating the slurry to 200° C., and secondly, introducing a high-pressure hydrogen into the slurry, wherein the total volume of the high-pressure hydrogen introduced twice and the slurry have a volume ratio of 1300:1; and heating the reaction raw material mixture to 340° C. and feeding it into a slurry bed reactor to undergo hydrolysis, cracking and hydrogenation reactions, and simultaneously introducing a cold hydrogen into the slurry bed reactor by controlling the slurry bed reactor to have a total gas velocity of 0.05 m/s; wherein, the high-pressure hydrogen has a pressure of 20 MPa, and the cold hydrogen has a temperature of 105° C.

The cold hydrogen is injected via 4 injection ports which are sequentially formed in a height direction in a side wall of the slurry bed reactor. The amorphous FeOOH used as a catalyst is stored in the slurry bed reactor in an amount of 9 wt % of the mass of liquid in the slurry bed reactor; and the reaction is carried out for a period of 40 min.

#### Embodiment 9

Provided is one-pot liquefaction process for biomass described as below.

##### Pretreatment of Biomass:

Soybean oil residue is fed into a drier for drying under a temperature of 95° C. for 3.5 h to have a moisture content

of less than 2 wt %, and then fed to an ultrafine pulverizer for initial pulverization to a median particle size of 110  $\mu\text{m}$ , then fed into a briquetting press for compressing at a temperature of 38° C. and a pressure of 2.5 MPa, and then extruded and molded, and then subjected to a second pulverization to produce a pretreated biomass having a median particle size of 50  $\mu\text{m}$  and a bulk density of 1500 kg/m<sup>3</sup>.

Preparation of Biomass Slurry:

The pretreated biomass is mixed with amorphous alumina (having a particle size of 200-500  $\mu\text{m}$ ) loading Mn oxide and Pd oxide, amorphous FeOOH and sulfur to obtain a mixture, and the mixture is added to water to carry out stirring grinding to form a slurry. The soybean oil residue is present in a total amount of 42 wt % in the slurry, and the slurry has a viscosity of 481 mPa·s (50° C.). Further, in the slurry, the total mass of amorphous alumina loading Mn oxide and Pd oxide and amorphous FeOOH accounts for 3 wt % and the vulcanizing agent accounts for 0.4 wt % of the mass of the pretreated biomass.

Liquefaction:

Introducing hydrogen into the slurry to carry out a reaction under a pressure of 20 MPa and a temperature of 420° C. to obtain a bio-oil.

Said introducing the high-pressure hydrogen into the slurry comprises two steps of: firstly, introducing a high-pressure hydrogen into the slurry till the volume ratio of the high-pressure hydrogen to the slurry is 100:1, and heating the slurry to 250° C., and secondly, introducing a high-pressure hydrogen into the slurry, wherein the total volume of the high-pressure hydrogen introduced twice and the slurry have a volume ratio of 1050:1; and heating the reaction raw material mixture to 420° C. and feeding it into a slurry bed reactor to undergo hydrolysis, cracking and hydrogenation reactions, and simultaneously introducing a cold hydrogen into the slurry bed reactor by controlling the slurry bed reactor to have a total gas velocity of 0.07 m/s; wherein, the high-pressure hydrogen has a pressure of 21 MPa, and the cold hydrogen has a temperature of 105° C.

The cold hydrogen is injected via 3 injection ports which are sequentially formed in a height direction in a side wall of the slurry bed reactor. The amorphous FeOOH as a catalyst is stored in the slurry bed reactor in an amount of 27 wt % of the mass of liquid in the slurry bed reactor; and the reaction is carried out for a period of 35 min.

Embodiment 10

Provided is one-pot liquefaction process for biomass described as below.

Pretreatment of Biomass:

Wheat straw is fed into a drier for drying under a temperature of 50° C. for 5 h to have a moisture content of less than 2 wt %, and then fed to an ultrafine pulverizer for initial pulverization to a median particle size of 100  $\mu\text{m}$ , then fed into a briquetting press for compressing at a temperature of 30° C. and a pressure of 3 MPa, and then extruded and molded, and then subjected to a second pulverization to produce a pretreated biomass having a median particle size of 30  $\mu\text{m}$  and a bulk density of 500 kg/m<sup>3</sup>.

Preparation of Catalyst:

S1, carrying out acidification on biomass charcoal to produce a biomass charcoal support; and.

S2, subjecting Mo oxide and the above biomass charcoal support to vibration grinding to obtain a biomass charcoal loading Mo oxide having a particle size of 400-500  $\mu\text{m}$ , i.e. a catalyst.

In the above catalyst, Mo accounts for 1% of the mass of the above biomass charcoal support. The acidification is carried out with an acid medium which has a H<sup>+</sup> concentration of 5 mol/L. A volume ratio of the carbonized biomass charcoal to the acid medium is 1:5, and the acidification is carried out at a temperature of 80° C. for a period of 1 h. Preparation of Biomass Slurry:

The pretreated biomass and the above catalyst are mixed with sulfur to obtain a mixture, and the mixture is added to a mixed oil of hogwash oil and residual oil to carry out stirring grinding to form a slurry. The wheat straw is present in a total amount of 55 wt % in the slurry, and the slurry has a viscosity of 500 mPa·s (50° C.). Further, in the slurry, the catalyst accounts for 1 wt %, and the vulcanizing agent accounts for 0.4 wt % of the mass of the pretreated biomass. Liquefaction:

Introducing hydrogen into the slurry to carry out a reaction under a pressure of 25 MPa and a temperature of 380° C. to obtain a bio-oil.

Said introducing hydrogen into the slurry comprises: introducing a high-pressure hydrogen into the slurry to prepare a reaction raw material mixture, wherein the high-pressure hydrogen and the slurry have a volume ratio of 1500:1; and heating the reaction raw material mixture to 380° C. and feeding it into a slurry bed reactor to undergo hydrolysis, cracking and hydrogenation reactions, and simultaneously introducing a cold hydrogen into the slurry bed reactor by controlling the slurry bed reactor to have a total gas velocity of 0.2 m/s; wherein, the high-pressure hydrogen has a pressure of 27 MPa, and the cold hydrogen has a temperature of 135° C.

The cold hydrogen is injected via 3 injection ports which are sequentially formed in a height direction in a side wall of the slurry bed reactor. The biomass charcoal loading Mo oxide as a catalyst is stored in the slurry bed reactor in an amount of 30 wt % of the mass of liquid in the slurry bed reactor; and the reaction is carried out for a period of 30 min.

Experimental Example

Results for evaluating the effects of the processes provided by the embodiments 1-9 are shown in table 1.

TABLE 1

| Product distributions of Embodiments 1-9 |              |                                                 |                            |                                        |                                                   |                                                     |                                                   |
|------------------------------------------|--------------|-------------------------------------------------|----------------------------|----------------------------------------|---------------------------------------------------|-----------------------------------------------------|---------------------------------------------------|
| Conversion results                       | Conversion % | Conver-<br>sion<br>rate of<br>bio-<br>mass<br>% | Yield<br>of oil<br>phase % | The<br>amount<br>of<br>residue<br>wt % | Carbo-<br>n<br>content<br>in oil<br>phase<br>wt % | Hydro-<br>gen<br>content<br>in oil<br>phase<br>wt % | Oxy-<br>gen<br>content<br>in oil<br>phase<br>wt % |
|                                          |              |                                                 |                            |                                        | in oil<br>phase<br>wt %                           | in oil<br>phase<br>wt %                             | in oil<br>phase<br>wt %                           |
| Embodiment 1                             | 99           | 76.0                                            | 0.07                       | 80                                     | 19                                                | 1.0                                                 |                                                   |
| Embodiment 2                             | 98           | 76.0                                            | 0.08                       | 83                                     | 14                                                | 3.0                                                 |                                                   |
| Embodiment 3                             | 96           | 79.5                                            | 0.09                       | 89                                     | 9.0                                               | 2.0                                                 |                                                   |
| Embodiment 4                             | 97           | 70                                              | 0.04                       | 80                                     | 18.1                                              | 1.9                                                 |                                                   |
| Embodiment 5                             | 97           | 75                                              | 0.09                       | 84                                     | 14                                                | 2                                                   |                                                   |
| Embodiment 6                             | 95           | 85                                              | 0.05                       | 89                                     | 10.5                                              | 0.5                                                 |                                                   |
| Embodiment 7                             | 98           | 60.0                                            | 0.07                       | 80                                     | 19                                                | 1                                                   |                                                   |
| Embodiment 8                             | 97           | 85.0                                            | 0.08                       | 90                                     | 9.9                                               | 0.1                                                 |                                                   |
| Embodiment 9                             | 95           | 86.0                                            | 0.09                       | 87                                     | 11.5                                              | 1.5                                                 |                                                   |

As shown in table 1, the conversion rate of biomass obtained by the method of the present invention is 95-99%, the yield of oil phase is 60-86%, the amount of residue is less than 0.1 wt %, the carbon content in oil phase is 80-90 wt %, the hydrogen content in oil phase is 9-19 wt %, and the oxygen content in oil phase is 0.1-3 wt %.

Provided is a method for preparing a second catalyst described as below.

S1, subjecting carbonized biomass charcoal to acidification or alkalization, thereby obtaining a second biomass charcoal support. Particularly, the acidification is carried out with an acid medium which has a H<sup>+</sup> concentration of 5 mol/L. A volume ratio of the carbonized biomass charcoal to the acid medium is 1:15, and the acidification is carried out at a temperature of 80° C. for a period of 10 h. The alkalization is carried out with an alkaline medium which has an OH concentration of 0.5 mol/L, and a volume ratio of the carbonized biomass charcoal to the alkaline medium is 1:5, and the alkalization is carried out at a temperature of 30° C. for a period of 10 h.

S2, subjecting a second active component and the second biomass charcoal support to vibration grinding and/or plane grinding and/or ball milling, thereby obtaining a second catalyst with a particle size of 100-200 µm.

The second active component is an oxide loading Mo and W, and based on mass of metal elements, the second active component accounts for 5% of the mass of the second biomass charcoal support.

Provided is a one-pot liquefaction process for biomass described as below.

(1) Corn straw is fed into a drier to be dried to have a moisture content of 3 wt %, and then fed to a pulverizer for pulverization to a particle size of 1-50 µm, and then removed dust to obtain straw particles.

(2) Amorphous alumina (having a particle size of 5-50 µm) loading Mo oxide and Co oxide is mixed with the straw particles obtained in the step (1) and sulfur uniformly according to a mass ratio of 5:100:0.3, thereby obtaining a mixture; and the mixture is added into medium/low temperature coal tar to form a slurry with a biomass content of 10 wt %.

(3) Firstly, introducing a high-pressure hydrogen having a pressure of 13 MPa and a temperature of 60° C. into the slurry till the volume ratio of the high-pressure hydrogen to the slurry is 50:1, and heating the slurry to 200° C. in a heat exchanger, and secondly, introducing a high-pressure hydrogen having a pressure of 13 MPa and a temperature of 200° C. into the slurry, wherein the total volume of the high-pressure hydrogen introduced twice and the slurry have a volume ratio of 800:1, obtaining a reaction raw material mixture; and heating the reaction raw material mixture to 450° C. and feeding it into a slurry bed reactor to undergo hydrolysis, cracking and hydrogenation reactions under a pressure of 13 MPa and a temperature of 500° C. During the reaction process, cold hydrogen with a temperature of 105° C. is introduced via 3 injection ports which are sequentially formed in a height direction in a side wall of the slurry bed reactor, wherein a total gas speed in the slurry bed reactor is controlled at 0.02 m/s, and the catalyst stored in the slurry bed reactor is controlled in an amount of 30 wt % of the total mass of the liquid phase and the solid phase in the slurry bed reactor. After reacting for 90 min, materials are discharged from the slurry bed reactor and are fed into a separation system to undergo gas, liquid and residue separation, thereby obtaining a biomass gas, a bio-oil and residues, respectively. The hydrogen in the reaction system is recycled

and is fed into each hydrogen injection site in the step (3) together with fresh supplementary hydrogen.

Provided is a one-pot liquefaction process for biomass described as below.

(1) Reeds are fed into a drier to be dried to have a moisture content of 5 wt %, and then fed to a pulverizer for pulverization to a particle size of 20-1000 µm, and then removed dust to obtain straw particles.

(2) Biomass charcoal (having a particle size of 100-150 µm) loading W oxide and Ni oxide is mixed with amorphous FeOOH, the reed particles obtained in the step (1) and sulfur uniformly according to a mass ratio of 2:2:100:0.4, thereby obtaining a mixture; and the mixture is added into vegetable oil, thereby obtaining a slurry with a biomass content of 30 wt %.

(3) Firstly, introducing a high-pressure hydrogen having a pressure of 20 MPa and a temperature of 70° C. into the slurry till the volume ratio of the high-pressure hydrogen to the slurry is 100:1, and heating the slurry to 250° C. in a heat exchanger, and secondly, introducing a high-pressure hydrogen having a pressure of 20 MPa and a temperature of 250° C. into the slurry, wherein the total volume of the high-pressure hydrogen introduced twice and the slurry have a volume ratio of 900:1, obtaining a reaction raw material mixture; and heating the reaction raw material mixture to 430° C. and feeding it into a slurry bed reactor to undergo hydrolysis, cracking and hydrogenation reactions under a pressure of 20 MPa and a temperature of 450° C. During the reaction process, cold hydrogen with a temperature of 120° C. is injected via 4 injection ports which are sequentially formed in a height direction in a side wall of the slurry bed reactor, wherein a total gas speed in the slurry bed reactor is controlled at 0.06 m/s, and the catalyst stored in the slurry bed reactor is controlled in an amount of 25 wt % of the total mass of the liquid phase and the solid phase in the slurry bed reactor. After reacting for 60 min, materials are discharged from the slurry bed reactor and are fed into a separation system to undergo gas, liquid and residue separation, thereby obtaining a biomass gas, a bio-oil and residues, respectively. The hydrogen in the reaction system is recycled and is fed into each hydrogen injection site in the step (3) together with fresh supplementary hydrogen.

Provided is a one-pot liquefaction process for biomass described as below.

(1) Wheat straw is fed into a drier to be dried to have a moisture content of 7 wt %, and then fed to a pulverizer for pulverization to a particle size of 1500-2000 µm, and then removed dust to obtain straw particles.

(2) Biomass charcoal (having a particle size of 50-100 µm) loading Pd oxide and Ni oxide is mixed with amorphous FeOOH, the straw particles obtained in the step (1) and sulfur uniformly according to a mass ratio of 2:3:100:0.3, thereby obtaining a mixture; and the mixture is added into low-temperature animal oil, thereby obtaining a slurry with a biomass content of 25 wt %.

(3) Firstly, introducing a high-pressure hydrogen having a pressure of 17 MPa and a temperature of 100° C. into the slurry till the volume ratio of the high-pressure hydrogen to the slurry is 150:1, and heating the slurry to 300° C. in a heat exchanger, and secondly, introducing a high-pressure hydrogen having a pressure of 17 MPa and a temperature of 300°

C. into the slurry, wherein the total volume of the high-pressure hydrogen introduced twice and the slurry have a volume ratio of 600:1, obtaining a reaction raw material mixture; and heating the reaction raw material mixture to 440° C. and feeding it into a slurry bed reactor to undergo hydrolysis, cracking and hydrogenation reactions under a pressure of 20 MPa and a temperature of 450° C. During the reaction process, cold hydrogen with a temperature of 90° C. is injected via 4 injection ports which are sequentially formed in a height direction in a side wall of the slurry bed reactor, wherein a total gas speed in the slurry bed reactor is controlled at 0.08 m/s, and the catalyst stored in the slurry bed reactor is controlled in an amount of 20 wt % of the total mass of the liquid phase and the solid phase in the slurry bed reactor. After reacting for 40 min, materials are discharged from the slurry bed reactor and are fed into a separation system to undergo gas, liquid and residue separation, thereby obtaining a biomass gas, a bio-oil and residues, respectively. The hydrogen in the reaction system is recycled and is fed into each hydrogen injection site in the step (3) together with fresh supplementary hydrogen.

## Embodiment 15

Provided is one-pot liquefaction process for biomass described as below.

(1) Wood chips are fed into a drier to be dried to have a moisture content of 10 wt %, and then fed to a pulverizer for pulverization to a particle size of 4000-5000  $\mu\text{m}$ , and then removed dust to obtain straw particles.

(2) Amorphous FeOOH (having a particle size of 150-200  $\mu\text{m}$ ) is mixed with the wood chip particles obtained in the step (1) and sulfur uniformly according to a mass ratio of 10:100:0.2, thereby obtaining a mixture; and the mixture is added into low-temperature animal oil to obtain a slurry with a biomass content of 40 wt %.

(3) Firstly, introducing a high-pressure hydrogen having a pressure of 27 MPa and a temperature of 130° C. into the slurry till the volume ratio of the high-pressure hydrogen to the slurry is 200:1, and heating the slurry to 350° C. in a heat exchanger, and secondly, introducing a high-pressure hydrogen having a pressure of 27 MPa and a temperature of 300° C. into the slurry, wherein the total volume of the high-pressure hydrogen introduced twice and the slurry have a volume ratio of 1000:1, obtaining a reaction raw material mixture; and heating the reaction raw material mixture to 300° C. and feeding it into a slurry bed reactor to undergo hydrolysis, cracking and hydrogenation reactions under a pressure of 27 MPa and a temperature of 300° C. During the reaction process, cold hydrogen with a temperature of 115° C. is injected via 5 injection ports which are sequentially formed in a height direction in a side wall of the slurry bed reactor, wherein a total gas speed in the slurry bed reactor is controlled at 0.1 m/s, and the catalyst stored in the slurry bed reactor is controlled in an amount of 30 wt % of the mass of the liquid phase in the slurry bed reactor. After reacting for 50 min, materials are discharged from the slurry bed reactor and are fed into a separation system to undergo gas, liquid and residue separation, thereby obtaining a biomass gas, a bio-oil and residues, respectively. The hydrogen in the reaction system is recycled and is fed into each hydrogen injection site in the step (3) together with fresh supplementary hydrogen.

## Embodiment 16

Provided is one-pot liquefaction process for biomass described as below.

(1) Leaves are fed into a drier to be dried to have a moisture content of 15 wt %, and then fed to a pulverizer for pulverization to a particle size of 4000-5000  $\mu\text{m}$ , and then removed dust to obtain leaves particles.

(2) The catalyst prepared in the embodiment 1 is mixed with amorphous FeOOH, the leaves particles obtained in the step (1) and sulfur uniformly according to a mass ratio of 1:0.2:100:0.25, thereby obtaining a mixture; and the mixture is added into low-temperature vegetable oil to obtain a slurry with a biomass content of 20 wt %.

(3) Firstly, introducing a high-pressure hydrogen having a pressure of 25 MPa and a temperature of 135° C. into the slurry till the volume ratio of the high-pressure hydrogen to the slurry is 200:1, and heating the slurry to 350° C. in a heat exchanger, and secondly, introducing a high-pressure hydrogen having a pressure of 25 MPa and a temperature of 350° C. into the slurry, wherein the total volume of the high-pressure hydrogen introduced twice and the slurry have a volume ratio of 650:1, obtaining a reaction raw material mixture; and heating the reaction raw material mixture to 400° C. and feeding it into a slurry bed reactor to undergo

hydrolysis, cracking and hydrogenation reactions under a pressure of 25 MPa and a temperature of 450° C. During the reaction process, cold hydrogen with a temperature of 100° C. is injected via 5 injection ports which are sequentially formed in a height direction in a side wall of the slurry bed reactor, wherein a total gas speed in the slurry bed reactor is controlled at 0.1 m/s, and the catalyst stored in the slurry bed reactor is controlled in an amount of 25 wt % of the mass of the liquid phase in the slurry bed reactor. After reacting for

15 20 25 30 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 9520 9525 9530 9535 9540 9545 9550 9555 9560 9565 9570 9575 9580 9585 9590 9595 9600 9605 9610 9615 9620 9625 9630 9635 9640 9645 9650 9655 9660 9665 9670 9675 9680 9685 9690 9695 9700 9705 9710 9715 9720 9725 9730 9735 9740 9745 9750 9755 9760 9765 9770 9

C. is injected via 4 injection ports which are sequentially formed in a height direction in a side wall of the slurry bed reactor, wherein a total gas speed in the slurry bed reactor is controlled at 0.06 m/s, and the catalyst stored in the slurry bed reactor is controlled in an amount of 25 wt % of the mass of the liquid phase in the slurry bed reactor. After reacting for 60 min, materials are discharged from the slurry bed reactor and are fed into a separation system to undergo gas, liquid and residue separation, thereby obtaining a biomass gas, a bio-oil and residues, respectively. The hydrogen in the reaction system is recycled and is fed into each hydrogen injection site in the step (3) together with fresh supplementary hydrogen.

#### Experimental Example

Results for evaluating the effects of the processes provided by the embodiments 12-16 and comparative example are shown in table 2.

As shown in table 2, the conversion rate of biomass and the yield of biomass oil of embodiments 12-16 are obviously higher than those of the comparative example, and residue content of embodiments 12-16 is obviously lower than that of the comparative example.

Carbon content and hydrogen content in the biomass oil of embodiments 12-16 are obviously higher than that of the comparative example, while oxygen content is obviously lower than that of the comparative example. By the comparison of embodiments 12-16 with the comparative example, the one-pot liquefaction process for biomass of the present invention is obviously superior to the existing liquefaction process for biomass.

TABLE 2

| Test item                             | Process effect |      |      |      |      |                     |
|---------------------------------------|----------------|------|------|------|------|---------------------|
|                                       | Embodiment No. |      |      |      |      |                     |
|                                       | 12             | 13   | 14   | 15   | 16   | Comparative example |
| Conversion rate of biomass %          | 95             | 92   | 90   | 91   | 99   | 80                  |
| Yield of biomass oil %                | 71             | 69   | 61   | 64   | 85.6 | 50                  |
| Residue content %                     | 0.06           | 0.03 | 0.04 | 0.04 | 0.01 | 2                   |
| Carbon content in the biomass oil %   | 86             | 88   | 87   | 85   | 87   | 75                  |
| Hydrogen content in the biomass oil % | 8.9            | 9.2  | 9.6  | 9.5  | 10.1 | 8.2                 |
| Oxygen content in the biomass oil %   | 4.1            | 2.4  | 2.8  | 4.8  | 2.1  | 16                  |

The following are embodiments of the one-pot liquefaction process for coal and biomass provided by the present invention. In each of the following embodiments and comparative examples, calculation formulas for conversion rate of biomass, yield of biomass oil, and residue content are as follows:

Conversion rate of coal and biomass=(the mass of liquefaction product-the mass of vulcanizing agent-mass of the catalyst-mass of the solvent oil)/the total mass of coal and biomass.

Yield of biomass oil=the mass of oil phase obtained after separation of the product of the liquefaction product/the total mass of coal and biomass.

Residue content=the mass of residue/the total mass of coal and biomass.

Provided is a method for preparing a second catalyst described as below.

#### 5 Preparation of Biomass Charcoal Support

Subjecting biomass charcoal to acidification by using an acid medium having a H<sup>+</sup> concentration of 5 mol/L at a temperature of 80° C. for a period of 10 h to obtain a biomass charcoal support, wherein the volume ratio of the acid medium to the biomass charcoal is 15:1. As an alternative, an alkaline medium having an OH<sup>-</sup> concentration of 0.5 mol/L can also be used for carrying out acidification to the biomass carbon at a volume ratio of 5:1 at 30° C. for 10 h.

#### 15 Loading a Second Active Component

Subjecting Mo oxide, W oxide and the above biomass charcoal support to vibration grinding to load active component onto the biomass charcoal support to obtain a second catalyst having a particle size of 100-200 μm. Based on mass 20 of metal elements, the second active component accounts for 5% of the mass of the biomass charcoal support.

25 Provided is one-pot liquefaction process for biomass and coal described as below.

#### Pretreatment of Straw

Corn straw is subjected to drying and dehydration to have a moisture content of less than 2 wt %, and then pulverized 30 to a median diameter of 100 μm, then sent to a plodder for extrusion molding under a molding pressure of 2 MPa to obtain a compressed straw material.

The compressed straw material is fed to a hammer mill for 35 pulverization to obtain pulverized straw material having a particle size of 50 μm.

#### Pretreatment of Coal Raw Material

Lignite is subjected to drying and dehydration, and then pulverized to a median diameter of 100 μm, then sent to a plodder for extrusion molding under a molding pressure of 5 MPa to obtain a compressed lignite material.

The compressed lignite material is sent to a ball mill for 40 pulverization to obtain pulverized lignite having a particle size of 30 μm.

#### 45 Preparation of Biomass Coal Slurry and Liquefaction Reaction

The above pulverized straw material and pulverized lignite are firstly subjected to dust removing, and then mixed with amorphous alumina (having a particle size of 5-50 μm) loading with Mo oxide and Co oxide and sulfur according to 50 a mass ratio of 100:5:0.3 to obtain a mixture, and the mixture is added to sour oil to form biomass coal slurry. In the biomass coal slurry, the straw has a content of 20 wt % and the lignite has a content of 45 wt %.

Introducing high-pressure hydrogen having a temperature 55 of 60° C. and a pressure of 15 MPa into the biomass coal slurry, wherein the volume of the introduced high-pressure hydrogen is 50 times the volume of the biomass coal slurry, and heating the slurry to 200° C. in a heat exchanger, and then introducing hydrogen having a pressure of 15 MPa and a temperature of 200° C. into the slurry, wherein the total 60 volume of the hydrogen introduced twice and the slurry have a volume ratio of 800:1, obtaining a reaction raw material mixture; and heating the reaction raw material mixture to 450° C. and feeding it into a slurry bed reactor to undergo

65 hydrolysis, cracking and hydrogenation reactions under a pressure of 15 MPa and a temperature of 460° C. During the reaction process, cold hydrogen with a temperature of 105°

C. is injected via 3 injection ports which are sequentially formed in a height direction in a side wall of the slurry bed reactor, wherein a total gas speed in the slurry bed reactor is controlled at 0.02 m/s, and the catalyst stored in the slurry bed reactor is controlled in an amount of 30 wt % of the mass of the liquid and solid phases in the slurry bed reactor. After reacting for 70 min, materials are discharged from the slurry bed reactor and are fed into a separation system to undergo gas, liquid and solid separation, thereby obtaining a biomass gas, a bio-oil and residues, respectively. The hydrogen in the reaction system is recycled and is fed into each hydrogen injection site mentioned above together with fresh supplementary hydrogen.

## Embodiment 19

Provided is one-pot liquefaction process for biomass and coal described as below.

## Pretreatment of Straw

Corn straw is subjected to drying and dehydration to have a moisture content of less than 1 wt %, and then pulverized to a median diameter of 100  $\mu\text{m}$ , then sent to a plodder for extrusion molding under a molding pressure of 2 MPa to obtain a compressed straw material.

The compressed straw material is sent to a hammer mill for pulverization to obtain pulverized straw material having a particle size of 50  $\mu\text{m}$ .

## Pretreatment of Coal Raw Material

Lignite is subjected to drying and dehydration, and then pulverized to a median diameter of 50  $\mu\text{m}$ , then sent to a plodder for extrusion molding under a molding pressure of 5 MPa to obtain a compressed lignite material.

The compressed lignite material is sent to a ball mill for pulverization to obtain pulverized lignite having a particle size of 30  $\mu\text{m}$ .

## Preparation of Biomass Water Coal Slurry and Liquefaction Reaction

The above pulverized straw material and pulverized lignite are firstly subjected to dust removing, and then mixed with amorphous alumina (having a particle size of 5-50  $\mu\text{m}$ ) loading with Mo oxide and Co oxide and sulfur according to a mass ratio of 100:5:0.3 to obtain a mixture, and the mixture is added to water to form biomass water coal slurry, wherein the straw has a content of 15 wt % and the lignite has a content of 40 wt %.

Introducing high-pressure hydrogen having a temperature of 60° C. and a pressure of 13 MPa into the resulting biomass water coal slurry, wherein the volume of the introduced high-pressure hydrogen is 50 times the volume of the slurry, and heating the slurry to 200° C. in a heat exchanger, and then introducing hydrogen having a pressure of 13 MPa and a temperature of 200° C. into the slurry, wherein the total volume of the hydrogen introduced twice and the slurry have a volume ratio of 800:1, obtaining a reaction raw material mixture; and heating the reaction raw material mixture to 450° C. and feeding it into a slurry bed reactor to undergo hydrolysis, cracking and hydrogenation reactions under a pressure of 15 MPa and a temperature of 300° C. During the reaction process, cold hydrogen with a temperature of 105° C. is injected via 3 injection ports which are sequentially formed in a height direction in a side wall of the slurry bed reactor, wherein a total gas speed in the slurry bed reactor is controlled at 0.02 m/s, and the catalyst stored in the slurry bed reactor is controlled in an amount of 30 wt % of the mass of the liquid and solid phases in the slurry bed reactor. After reacting for 60 min, materials are discharged from the slurry bed reactor and are fed into a separation system to undergo gas, liquid and residue separation, thereby obtaining a biomass gas, a bio-oil and residues, respectively. The hydrogen in the reaction

ration system to undergo gas, liquid and solid separation, thereby obtaining a biomass gas, a bio-oil and residues, respectively. The hydrogen in the reaction system is recycled and is fed into each hydrogen injection site mentioned above together with fresh supplementary hydrogen.

## Embodiment 20

Provided is one-pot liquefaction process for biomass and coal described as below.

## Pretreatment of Biomass Materials:

(1) Reeds are dried to have a moisture content of 1 wt %, and then fed to a pulverizer for pulverization to obtain a first reed pulverized material having a particle size  $D_{50}$  of 200  $\mu\text{m}$ .

(2) The first reed pulverized material is sent to a briquetting press or a plodder for extrusion molding under a molding pressure of 3 MPa to obtain reeds compressed materials.

(3) The reeds compressed materials are fed to a pulverizer for second pulverization to obtain a second reed pulverized material having a particle size  $D_{50}$  of 40  $\mu\text{m}$ .

## Pretreatment of Coal Raw Material:

(1) Shendong long flame coal is subjected to drying and dehydration, and then fed to a ball mill for pulverization to obtain a first pulverized material having a particle size  $D_{50}$  of 50  $\mu\text{m}$ .

(2) The first pulverized material is sent to a briquetting press or a plodder for extrusion molding under a molding pressure of 12 MPa to obtain compressed materials.

(3) The compressed materials are fed to a pulverizer for a second pulverization to obtain a second pulverized material having a particle size  $D_{50}$  of 80  $\mu\text{m}$ .

## Preparation of Biomass Water Coal Slurry and Liquefaction Reaction

The second pulverized reed material and the second pulverized coal material are mixed with biomass charcoal (having a particle size of 100-150  $\mu\text{m}$ ) loading W oxide and Ni oxide, FeOOH, and sulfur uniformly according to a mass ratio of 100:2:2:0.4, thereby obtaining a mixture; and the mixture is added into water, thereby obtaining a biomass water coal slurry with a reed content of 20 wt % and a coal content of 40 wt %.

Introducing a high-pressure hydrogen having a pressure of 20 MPa and a temperature of 70° C. into the slurry till the volume ratio of the high-pressure hydrogen to the slurry is 100:1, and heating the slurry to 250° C. in a heat exchanger, and then introducing hydrogen having a pressure of 20 MPa and a temperature of 250° C. into the slurry, wherein the total volume of the high-pressure hydrogen introduced twice and the slurry have a volume ratio of 900:1, obtaining a reaction raw material mixture; and heating the reaction raw material mixture to 430° C. and feeding it into a slurry bed reactor to undergo hydrolysis, cracking and hydrogenation reactions under a pressure of 20 MPa and a temperature of 450° C. During the reaction process, cold hydrogen with a temperature of 120° C. is injected via 4 injection ports which are sequentially formed in a height direction in a side wall of the slurry bed reactor, wherein a total gas speed in the slurry bed reactor is controlled at 0.06 m/s, and the catalyst stored in the slurry bed reactor is controlled in an amount of 25 wt % of the total mass of the liquid phase and the solid phase in the slurry bed reactor. After reacting for 60 min, materials are discharged from the slurry bed reactor and are fed into a separation system to undergo gas, liquid and residue separation, thereby obtaining a biomass gas, a bio-oil and residues, respectively. The hydrogen in the reaction

35

system is recycled and is fed into each hydrogen injection site mentioned above together with fresh supplementary hydrogen.

## Embodiment 21

Provided is one-pot liquefaction process for biomass and coal described as below.

## Pretreatment of Biomass and Coal Raw Material:

Palm oil residue and lignite are subjected to drying and dehydration, and then fed to a briquetting press for extrusion molding under a molding pressure of 5 MPa to obtain compressed materials of palm oil residue and lignite, which are then fed to a ball mill for pulverization to obtain a pulverized material of palm oil residue and lignite having a median diameter of 50  $\mu\text{m}$ .

## Preparation of Biomass Water Coal Slurry and Hydrolysis Hydrogenation Reaction

The above pulverized material is mixed with amorphous alumina (having a particle size of 350-500  $\mu\text{m}$ ) loading Mo oxide and Ni oxide and sulfur uniformly according to a mass ratio of 100:1:0.1, thereby obtaining a mixture; and the mixture is added into water, thereby obtaining a biomass water coal slurry with a palm oil residue content of 20 wt % and a coal content of 45 wt %.

Introducing a high-pressure hydrogen having a pressure of 20 MPa and a temperature of 90° C. into the slurry till the volume ratio of the high-pressure hydrogen to the slurry is 150:1, and heating the slurry to 300° C. in a heat exchanger, and then introducing hydrogen having a pressure of 20 MPa and a temperature of 300° C. into the slurry, wherein the total volume of the high-pressure hydrogen introduced twice and the slurry have a volume ratio of 800:1, obtaining a reaction raw material mixture; and heating the reaction raw material mixture to 430° C. and feeding it into a slurry bed reactor to undergo hydrolysis, cracking and hydrogenation reactions under a pressure of 20 MPa and a temperature of 460° C. During the reaction process, cold hydrogen with a temperature of 120° C. is injected via 5 injection ports which are sequentially formed in a height direction in a side wall of the slurry bed reactor, wherein a total gas speed in the slurry bed reactor is controlled at 0.07 m/s, and the catalyst stored in the slurry bed reactor is controlled in an amount of 30 wt % of the total mass of the liquid phase in the slurry bed reactor. After reacting for 40 min, materials are discharged from the slurry bed reactor and are fed into a separation system to undergo gas, liquid and residue separation, thereby obtaining a biomass gas, a bio-oil and residues, respectively. The hydrogen in the reaction system is recycled and is fed into each hydrogen injection site mentioned above together with fresh supplementary hydrogen.

## Embodiment 22

Provided is one-pot liquefaction process for coal and biomass described as below.

## Pretreatment of Biomass Materials:

(1) Soybean oil residue is subjected to drying and dehydration, and then fed to a pulverizer for a first pulverization to obtain a first pulverized material of soybean oil residue having a particle size  $D_{50}$  of 250  $\mu\text{m}$ .

(2) The first pulverized material is sent to a briquetting press or a plodder for extrusion molding under a molding pressure of 5 MPa to obtain a compressed material of soybean oil residue.

36

(3) The compressed material is fed to a pulverizer for a second pulverization to obtain a second pulverized material of soybean oil residue having a particle size  $D_{50}$  of 45  $\mu\text{m}$ .

## Pretreatment of Coal Raw Material

(1) Shendong long flame coal is subjected to drying and dehydration, and then fed to a ball mill for pulverization to obtain a first pulverized material having a particle size  $D_{50}$  of 60  $\mu\text{m}$ .

(2) The first pulverized material is sent to a briquetting press or a plodder for extrusion molding under a molding pressure of 10 MPa to obtain a compressed material.

(3) The compressed material is fed to a ball mill for carrying out a second pulverization to obtain a second pulverized material having a particle size  $D_{50}$  of 40  $\mu\text{m}$ .

## Preparation of Biomass Coal Slurry and Liquefaction Reaction

The present embodiment adopts a catalyst prepared by embodiment 1. The second pulverized material of soybean oil residue and the second pulverized material of coal are uniformly mixed with the above catalyst, FeOOH, and sulfur according to a mass ratio of 100:1:0.2:0.25, thereby obtaining a mixture; and the mixture is added into a waste lubricating oil, thereby obtaining a biomass coal slurry with a soybean oil residue content of 20 wt % and a coal content of 40 wt %.

Introducing a high-pressure hydrogen having a pressure of 25 MPa and a temperature of 135° C. into the slurry till the volume ratio of the high-pressure hydrogen to the slurry is 200:1, and heating the slurry to 350° C. in a heat exchanger, and then introducing hydrogen having a pressure of 25 MPa and a temperature of 350° C. into the slurry, wherein the total volume of the high-pressure hydrogen introduced twice and the slurry have a volume ratio of 650:1, obtaining a reaction raw material mixture; and heating the reaction raw material mixture to 400° C. and feeding it into a slurry bed reactor to undergo hydrolysis, cracking and hydrogenation reactions under a pressure of 25 MPa and a temperature of 450° C. During the reaction process, cold hydrogen with a temperature of 100° C. is injected via 5 injection ports which are sequentially formed in a height direction in a side wall of the slurry bed reactor, wherein a total gas speed in the slurry bed reactor is controlled at 0.1 m/s, and the catalyst stored in the slurry bed reactor is controlled in an amount of 25 wt % of the total mass of the liquid phase in the slurry bed reactor. After reacting for 15 min, materials are discharged from the slurry bed reactor and are fed into a separation system to undergo gas, liquid and residue separation, thereby obtaining a biomass gas, a bio-oil and residues, respectively. The hydrogen in the reaction system is recycled and is fed into each hydrogen injection site mentioned above together with fresh supplementary hydrogen.

55

## Embodiment 23

Provided is one-pot liquefaction process for coal and biomass described as below.

## Pretreatment of Biomass and Coal Raw Material:

Palm oil residue and lignite are subjected to drying and dehydration to have a moisture content of less than 2 wt %, and then fed to a briquetting press for extrusion molding under a molding pressure of 5 MPa to obtain a compressed material of palm oil residue and lignite, which is then fed to a ball mill for pulverization to obtain a pulverized material of palm oil residue and lignite.

Preparation of Biomass Water Coal Slurry and Liquefaction Hydrogenation Reaction

The above pulverized material is mixed uniformly with amorphous alumina (having a particle size of 350-500  $\mu\text{m}$ ) loading Mo oxide and Ni oxide, and sulfur according to a mass ratio of 100:1:0.1, thereby obtaining a mixture; and the mixture is added into gutter oil, thereby obtaining a biomass water coal slurry with a palm oil residue content of 25 wt % and a coal content of 40 wt %.

Introducing a high-pressure hydrogen having a pressure of 20 MPa and a temperature of 90° C. into the slurry till the volume ratio of the high-pressure hydrogen to the slurry is 150:1, and heating the slurry to 300° C. in a heat exchanger, and then introducing hydrogen having a pressure of 20 MPa and a temperature of 300° C. into the slurry, wherein the total volume of the high-pressure hydrogen introduced twice and the slurry have a volume ratio of 800:1, obtaining a reaction raw material mixture; and heating the reaction raw material mixture to 430° C. and feeding it into a slurry bed reactor to undergo hydrolysis, cracking and hydrogenation reactions under a pressure of 20 MPa and a temperature of 420° C. During the reaction process, cold hydrogen with a temperature of 120° C. is injected via 5 injection ports which are sequentially formed in a height direction in a side wall of the slurry bed reactor, wherein a total gas speed in the slurry bed reactor is controlled at 0.07 m/s, and the catalyst stored in the slurry bed reactor is controlled in an amount of 40 wt % of the total mass of the liquid phase in the slurry bed reactor. After reacting for 40 min, materials are discharged from the slurry bed reactor and are fed into a separation system to undergo gas, liquid and residue separation, thereby obtaining a biomass gas, a bio-oil and residues, respectively. The hydrogen in the reaction system is recycled and is fed into each hydrogen injection site mentioned above together with fresh supplementary hydrogen.

Embodiment 24

Provided is one-pot liquefaction process for coal and biomass described as below.

Pretreatment of Biomass Raw Material:

(1) Reeds are dried to have a moisture content of 1 wt %, and then fed to a pulverizer for pulverization to obtain a first reed pulverized material having a particle size  $D_{50}$  of 300  $\mu\text{m}$ .

(2) The first reed pulverized material is sent to a briquetting press or a plodder for extrusion molding under a molding pressure of 5 MPa to obtain a compressed reed material.

(3) The compressed reed material is fed to a pulverizer for a second pulverization to obtain a second pulverized material of reed having a particle size  $D_{50}$  of 30  $\mu\text{m}$ .

Pretreatment of Coal Raw Material:

(1) Shendong long flame coal is subjected to drying and dehydration, and then fed to a ball mill for pulverization to obtain a first pulverized material having a particle size  $D_{50}$  of 50  $\mu\text{m}$ .

(2) The first pulverized material is sent to a briquetting press or a plodder for extrusion molding under a molding pressure of 15 MPa to obtain a compressed material.

(3) The compressed material is fed to a ball mill for a second pulverization to obtain a second pulverized material having a particle size  $D_{50}$  of 45  $\mu\text{m}$ .

Preparation of Biomass Coal Slurry and Liquefaction Reaction

The second pulverized material of reeds and coal is mixed with biomass charcoal (having a particle size of 100-150  $\mu\text{m}$ ) loading W oxide and Ni oxide, FeOOH, and sulfur

uniformly according to a mass ratio of 100:2:2:0.4, thereby obtaining a mixture; and the mixture is added into a waste engine oil, thereby obtaining a biomass coal slurry with a reed content of 30 wt % and a coal content of 30 wt %.

Introducing a high-pressure hydrogen having a pressure of 17 MPa and a temperature of 70° C. into the slurry till the volume ratio of the high-pressure hydrogen to the slurry is 100:1, and heating the slurry to 250° C. in a heat exchanger, and then introducing hydrogen having a pressure of 17 MPa and a temperature of 250° C. into the slurry, wherein the total volume of the high-pressure hydrogen introduced twice and the slurry have a volume ratio of 900:1, obtaining a reaction raw material mixture; and heating the reaction raw material mixture to 430° C. and feeding it into a slurry bed reactor to undergo hydrolysis, cracking and hydrogenation reactions under a pressure of 17 MPa and a temperature of 450° C. During the reaction process, cold hydrogen with a temperature of 120° C. is injected via 4 injection ports which are sequentially formed in a height direction in a side wall of the slurry bed reactor, wherein a total gas speed in the slurry bed reactor is controlled at 0.06 m/s, and the catalyst stored in the slurry bed reactor is controlled in an amount of 25 wt % of the total mass of the liquid phase and the solid phase in the slurry bed reactor. After reacting for 60 min, materials are discharged from the slurry bed reactor and are fed into a separation system to undergo gas, liquid and residue separation, thereby obtaining a biomass gas, a bio-oil and residues, respectively. The hydrogen in the reaction system is recycled and is fed into each hydrogen injection site mentioned above together with fresh supplementary hydrogen.

Comparative Example 1

Provided is comparative one-pot liquefaction process for coal and biomass described as below.

Pretreatment of Biomass Raw Material:

(1) Reeds are fed into a drier to have a moisture content of 1.5 wt %, and then fed to a pulverizer for pulverization to obtain a first reed pulverized material having a particle size  $D_{50}$  of 200  $\mu\text{m}$ .

(2) The first reed pulverized material is sent to a briquetting press or a plodder for extrusion molding under a molding pressure of 3 MPa to obtain a reed compressed material.

(3) The reed compressed material is fed to a pulverizer for a second pulverization to obtain a second reed pulverized material having a particle size  $D_{50}$  of 40  $\mu\text{m}$ .

Pretreatment of Coal Raw Material:

(1) Shendong long flame coal is subjected to drying and dehydration, and then fed to a ball mill for pulverization to obtain a first pulverized material having a particle size  $D_{50}$  of 80  $\mu\text{m}$ .

(2) The first pulverized material is sent to a briquetting press or a plodder for extrusion molding under a molding pressure of 12 MPa to obtain a compressed material.

(3) The compressed material is fed to a ball mill for a second pulverization to obtain a second pulverized material having a particle size  $D_{50}$  of 80  $\mu\text{m}$ .

Preparation of Biomass Water Coal Slurry and Liquefaction Reaction

The second pulverized material of reeds and coal is mixed with water-soluble dispersive hydrogenation catalyst after vulcanization uniformly according to a mass ratio of 100:4.4, thereby obtaining a mixture; and the mixture is added into water, thereby obtaining a biomass water coal slurry with a reed content of 20 wt % and a coal content of 45 wt %.

Introducing a high-pressure hydrogen having a pressure of 20 MPa and a temperature of 70° C. into the slurry till the volume ratio of the high-pressure hydrogen to the slurry is 100:1, and heating the slurry to 250° C. in a heat exchanger, and then introducing hydrogen having a pressure of 20 MPa and a temperature of 250° C. into the slurry, wherein the total volume of the high-pressure hydrogen introduced twice and the slurry have a volume ratio of 900:1, obtaining a reaction raw material mixture; and heating the reaction raw material mixture to 430° C. and feeding it into a slurry bed reactor to undergo hydrolysis, cracking and hydrogenation reactions under a pressure of 20 MPa and a temperature of 450° C. During the reaction process, cold hydrogen with a temperature of 120° C. is injected via 4 injection ports which are sequentially formed in a height direction in a side wall of the slurry bed reactor, wherein a total gas speed in the slurry bed reactor is controlled at 0.06 m/s, and the catalyst stored in the slurry bed reactor is controlled in an amount of 25 wt % of the total mass of the liquid phase and the solid phase in the slurry bed reactor. After reacting for 60 min, materials are discharged from the slurry bed reactor and are fed into a separation system to undergo gas, liquid and residue separation, thereby obtaining a biomass gas, a bio-oil and residues, respectively. The hydrogen in the reaction system is recycled and is fed into each hydrogen injection site mentioned above together with fresh supplementary hydrogen.

#### Comparative Example 2

Provided is comparative one-pot liquefaction process for coal and biomass described as below.

##### Pretreatment of Biomass Raw Material:

(1) Reeds are fed into a drier to have a moisture content of 1 wt %, and then fed to a pulverizer for pulverization to obtain a first reed pulverized material having a particle size  $D_{50}$  of 300  $\mu\text{m}$ .

(2) The first reed pulverized material is sent to a briquetting press or a plodder for extrusion molding under a molding pressure of 5 MPa to obtain a reed compressed material.

(3) The reed compressed material is fed to a pulverizer for a second pulverization to obtain a second reed pulverized material having a particle size  $D_{50}$  of 30  $\mu\text{m}$ .

(3) The compressed material is fed to a ball mill for a second pulverization to obtain a second pulverized material having a particle size  $D_{50}$  of 45  $\mu\text{m}$ .

##### Preparation of Biomass Coal Slurry and Liquefaction Reaction

The second pulverized material of reeds and coal is mixed with water-soluble dispersive hydrogenation catalyst after vulcanization uniformly according to a mass ratio of 100:2, thereby obtaining a mixture; and the mixture is added into waste engine oil, thereby obtaining a biomass coal slurry with a reed content of 30 wt % and a coal content of 30 wt %.

Introducing a high-pressure hydrogen having a pressure of 17 MPa and a temperature of 70° C. into the slurry till the volume ratio of the high-pressure hydrogen to the slurry is 100:1, and heating the slurry to 250° C. in a heat exchanger, and then introducing hydrogen having a pressure of 17 MPa and a temperature of 250° C. into the slurry, wherein the total volume of the high-pressure hydrogen introduced twice and the slurry have a volume ratio of 900:1, obtaining a reaction raw material mixture; and heating the reaction raw material mixture to 430° C. and feeding it into a slurry bed reactor to undergo hydrolysis, cracking and hydrogenation reactions under a pressure of 17 MPa and a temperature of 450° C. During the reaction process, cold hydrogen with a temperature of 120° C. is injected via 4 injection ports which are sequentially formed in a height direction in a side wall of the slurry bed reactor, wherein a total gas speed in the slurry bed reactor is controlled at 0.06 m/s, and the catalyst stored in the slurry bed reactor is controlled in an amount of 25 wt % of the total mass of the liquid phase and the solid phase in the slurry bed reactor. After reacting for 60 min, materials are discharged from the slurry bed reactor and are fed into a separation system to undergo gas, liquid and residue separation, thereby obtaining a biomass gas, a bio-oil and residues, respectively. The hydrogen in the reaction system is recycled and is fed into each hydrogen injection site mentioned above together with fresh supplementary hydrogen.

Results for evaluating the effects of the processes provided by the embodiments 18-24 and comparative examples are shown in table 3.

TABLE 3

| Item                                             | Process effect |     |    |     |    |     |     |                       | Embodiment No.        |   |
|--------------------------------------------------|----------------|-----|----|-----|----|-----|-----|-----------------------|-----------------------|---|
|                                                  | 18             | 19  | 20 | 21  | 22 | 23  | 24  | Comparative example 1 | Comparative example 2 |   |
| Conversion rate (%)                              | 93             | 95  | 92 | 93  | 94 | 99  | 96  | 79                    | 76                    |   |
| Yield of biomass oil (%)                         | 79             | 79  | 76 | 85  | 73 | 95  | 80  | 49                    | 53                    |   |
| Residue content (%)                              | 0.8            | 0.4 | 2  | 0.3 | 1  | 0.3 | 1   | 10                    | 5                     |   |
| Main element content of the resulting oil (wt %) | C              | 90  | 86 | 90  | 87 | 87  | 86  | 65                    | 69                    |   |
|                                                  | H              | 8   | 7  | 6   | 10 | 10  | 7   | 5                     | 8                     |   |
|                                                  | O              | 0.5 | 1  | 2   | 1  | 0.9 | 1.5 | 1.5                   | 7                     | 6 |

##### Pretreatment of Coal Raw Material:

(1) Shendong long flame coal is subjected to drying and dehydration, and then fed to a ball mill for pulverization to obtain a first pulverized material having a particle size  $D_{50}$  of 50  $\mu\text{m}$ .

(2) The first pulverized material is sent to a briquetting press or a plodder for extrusion molding under a molding pressure of 15 MPa to obtain a compressed material.

As shown in table 3, when choosing different catalysts, the conversion rate of biomass and the yield of biomass oil of embodiments 18-24 are obviously higher than that of the comparative examples 1 and 2, and residue content of embodiments 18-24 is obviously lower than that of the comparative examples 1 and 2.

Apparently, the aforementioned embodiments are merely examples illustrated for clearly describing the present invention.

tion, rather than limiting the implementation ways thereof. For those skilled in the art, various changes and modifications in other different forms can be made on the basis of the aforementioned description. It is unnecessary and impossible to exhaustively list all the implementation ways herein. However, any obvious changes or modifications derived from the aforementioned description are intended to be embraced within the protection scope of the present invention.

We claim:

1. Process for one-pot liquefaction of biomass, comprising the following steps:

preparing a slurry containing a catalyst, a vulcanizing agent and a biomass, and introducing hydrogen into the slurry to carry out a reaction under a pressure of 15-25 MPa and a temperature of 380-480° C., thereby obtaining a bio-oil;

wherein, the slurry is prepared with using straw as the biomass according to the following steps: subjecting the straw sequentially to drying, a first pulverization, compression and a second pulverization to obtain a pretreated biomass, and then mixing the pretreated biomass with the catalyst and the vulcanizing agent to obtain a mixture, and adding the mixture to an oil to carry out grinding pulping to obtain the slurry having a straw concentration of 30 wt % to 60 wt %.

2. The process according to claim 1, wherein, said subjecting the straw to compression is carried out under a pressure of 0.5-3 MPa and a temperature of 30-60° C.

3. The process according to claim 1, wherein, said subjecting the straw to drying is carried out at a temperature of 50-70° C. for a period of 3-5 h to obtain a dried straw having a moisture content of less than 2 wt %, and after the first pulverization the dried straw has a median particle size of 100-300 µm, and after the second pulverization the dried straw has a median particle size of 30-50 µm and a bulk density of 400-500 kg/m<sup>3</sup>.

4. The process according to claim 1, wherein the slurry has a straw content of 55-60 wt %.

5. Process for one-pot liquefaction of biomass according to claim 1, comprising the following steps:

preparing a slurry containing a catalyst, a vulcanizing agent and a biomass, and introducing hydrogen into the slurry to carry out a reaction under a pressure of 15-25 MPa and a temperature of 380-480° C., thereby obtaining a bio-oil;

wherein, the slurry is prepared with using a vegetable oil residue as the biomass according to the following steps: subjecting the vegetable oil residue sequentially to drying, a first pulverization, compression and a second pulverization to obtain a pretreated biomass, and then mixing the pretreated biomass with the catalyst and the vulcanizing agent to obtain a mixture, and adding the mixture to an oil to carry out grinding pulping to obtain the slurry having a vegetable oil residue concentration of 50 wt % to 65 wt %.

6. The process according to claim 5, wherein, said subjecting the vegetable oil residue to compression is carried out under a pressure of 3-5 MPa and a temperature of 40-60° C.

7. The process according to claim 5, wherein, said subjecting the vegetable oil residue to drying is carried out at a temperature of 80-110° C. for a period of 2-6 h to obtain a dried vegetable oil residue having a moisture content of less than 2 wt %, and after the first pulverization the dried vegetable oil residue has a median particle size of 100-300

µm, and after the second pulverization the dried vegetable oil residue has a median particle size of 30-50 µm and a bulk density of 1500-1600 kg/m<sup>3</sup>.

8. The process according to claim 1, wherein, the oil is selected from the group consisting of waste animal and vegetable oil, waste mineral oil, mineral oil, distillate oil, and any combination thereof.

9. Process for one-pot liquefaction of biomass, comprising the following steps:

10. preparing a slurry containing a catalyst, a vulcanizing agent and a biomass, and introducing hydrogen into the slurry to carry out a reaction under a pressure of 15-20 MPa and a temperature of 300-400° C., thereby obtaining a bio-oil;

wherein, the slurry is prepared with using straw as the biomass according to the following steps: subjecting the straw sequentially to drying, a first pulverization, compression and a second pulverization to obtain a pretreated biomass, and then mixing the pretreated biomass with the catalyst and the vulcanizing agent to obtain a mixture, and adding the mixture to water to carry out grinding pulping to obtain the slurry having a straw concentration of 35 to 50 wt %.

10. The process according to claim 9, wherein said subjecting the straw to the compression is carried out at under a pressure of 2-5 MPa and a temperature of 30-60° C.

11. The process according to claim 9, wherein, said subjecting the straw to drying is carried out at a temperature of 70-110° C. for a period of 3-5 h to obtain a dried straw having a moisture content of less than 2 wt %, and after the first pulverization the dried straw has a median particle size of 100-300 µm, and after the second pulverization the dried straw has a median particle size of 30-50 µm and a bulk density of 400-800 kg/m<sup>3</sup>.

12. Process for one-pot liquefaction of biomass, comprising the following steps:

preparing a slurry containing a catalyst, a vulcanizing agent and a biomass, and introducing hydrogen into the slurry to carry out a reaction under a pressure of 15-20 MPa and a temperature of 340-420° C., thereby obtaining a bio-oil;

wherein the slurry is prepared with using a vegetable oil residue as the biomass according to the following steps: subjecting the vegetable oil residue sequentially to drying, a first pulverization, compression and a second pulverization to obtain a pretreated biomass, and then mixing the pretreated biomass with the catalyst and the vulcanizing agent to obtain a mixture, and adding the mixture to water to carry out grinding pulping to obtain the slurry having a vegetable oil residue concentration of 40 to 50 wt %.

13. The process according to claim 12, wherein, said subjecting the vegetable oil residue to compression is carried out under a pressure of 0.5-3 MPa and a temperature of 30-50° C.

14. The process according to claim 12, wherein, said subjecting the vegetable oil residue to drying is carried out at a temperature of 80-110° C. for a period of 2-6 h to obtain a dried vegetable oil residue having a moisture content of less than 2 wt %, and after the first pulverization the dried vegetable oil residue has a median particle size of 50-300 µm, and after the second pulverization the dried vegetable oil residue has a median particle size of 30-50 µm and a bulk density of 1400-1600 kg/m<sup>3</sup>.

15. The process according to claim 1, wherein the catalyst is selected from the group consisting of amorphous FeOOH, amorphous alumina loading an active component, biomass

charcoal loading an active component, and any combination thereof, and wherein the active component is selected from the group consisting of oxides of metals of group VIIB, group VIIIB, group VIII, and any combination thereof in the periodic table of elements.

16. The process according to claim 15, wherein, the active component is selected from the group consisting of oxides of Mo, W, Fe, Co, Ni, Mn, Pd, and any combination thereof.

17. The process according to claim 1, wherein the catalyst is present in an amount of 1-10 wt % of the mass of the pretreated biomass, and has a particle size of 5-500  $\mu\text{m}$ ; and the vulcanizing agent is present in an amount of 0.1-0.4 wt % of the mass of the pretreated biomass.

18. The process according to claim 1, wherein, said introducing hydrogen into the slurry comprises:

introducing a high-pressure hydrogen into the slurry to prepare a reaction raw material mixture, wherein the high-pressure hydrogen and the slurry have a volume ratio of (600-1500):1; and

heating the reaction raw material mixture to 380-480° C. and feeding it into a slurry bed reactor to undergo hydrolysis, cracking and hydrogenation reactions, and simultaneously introducing a cold hydrogen into the slurry bed reactor by controlling the slurry bed reactor to have a total gas velocity of 0.02-0.2 m/s, preferably 0.05-0.08 m/s;

wherein, the high-pressure hydrogen has a pressure of 15-27 MPa, and the cold hydrogen has a temperature of 60-135° C.

19. The process according to claim 18, wherein said introducing the high-pressure hydrogen into the slurry comprises two steps of:

firstly, introducing a high-pressure hydrogen into the slurry till the volume ratio of the high-pressure hydrogen to the slurry is (50-200):1, and heating the slurry to 200-350° C., and

secondly, introducing a high-pressure hydrogen into the slurry.

20. The process according to claim 18, wherein, the catalyst stored in the slurry bed reactor is controlled in an amount of 5-30 wt % of the mass of liquid phase in the slurry bed reactor; and

the reaction is carried out for a period of 30-120 min.

21. The process according to claim 9, wherein, said introducing hydrogen into the slurry comprises:

introducing a high-pressure hydrogen into the slurry to prepare a reaction raw material mixture, wherein the high-pressure hydrogen and the slurry have a volume ratio of (600-1500):1; and

heating the reaction raw material mixture to 300-400° C. and feeding it into a slurry bed reactor to undergo hydrolysis, cracking and hydrogenation reactions, and simultaneously introducing a cold hydrogen into the slurry bed reactor by controlling the slurry bed reactor to have a total gas velocity of 0.02-0.2 m/s, preferably 0.05-0.08 m/s;

wherein, the high-pressure hydrogen has a pressure of 15-22 MPa, and the cold hydrogen has a temperature of 60-135° C.

22. The process according to claim 12, wherein, said introducing hydrogen into the slurry comprises:

introducing a high-pressure hydrogen into the slurry to prepare a reaction raw material mixture, wherein the high-pressure hydrogen and the slurry have a volume ratio of (600-1500):1; and

heating the reaction raw material mixture to 340-420° C. and feeding it into a slurry bed reactor to undergo

hydrolysis, cracking and hydrogenation reactions, and simultaneously introducing a cold hydrogen into the slurry bed reactor by controlling the slurry bed reactor to have a total gas velocity of 0.02-0.2 m/s;

5 wherein, the high-pressure hydrogen has a pressure of 15-22 MPa, and the cold hydrogen has a temperature of 60-135° C.

23. The process according to claim 21, wherein, said introducing the high-pressure hydrogen into the slurry comprises two steps of:

firstly, introducing a high-pressure hydrogen into the slurry till the volume ratio of the high-pressure hydrogen to the slurry is (50-200):1, and heating the slurry to 200-280° C., and

secondly, introducing a high-pressure hydrogen into the slurry.

24. The process according to claim 21, wherein, the catalyst stored in the slurry bed reactor is controlled in an amount of 5-30 wt % of the mass of liquid phase in the slurry bed reactor; and

the reaction is carried out for a period of 30-60 min.

25. Process for one-pot liquefaction of biomass, comprising the following steps:

preparing a biomass coal slurry by mixing a biomass powder, a coal powder, a catalyst, and a vulcanizing agent with a flowing medium, and perform grinding pulping, wherein the flowing medium is an oil or water; and wherein the biomass powder is prepared by collecting a biomass and controlling the biomass to have a moisture content of less than 2 wt %, then pulverizing the biomass to a median particle size of 100-300  $\mu\text{m}$ , compressing and molding the pulverized biomass under a pressure of 2-5 MPa and a temperature of 30-60° C., and pulverizing the compressed biomass again to a median particle size of 30-50  $\mu\text{m}$ ; and wherein the coal powder is prepared by collecting a coal and controlling the coal to have a moisture content of less than 2 wt %, then pulverizing it to a median particle size of 50-100  $\mu\text{m}$  under a temperature of 30-60° C., compressing and molding the pulverized coal under a pressure of 5-15 MPa, and pulverizing the compressed coal again;

carrying out a liquefaction reaction, comprising introducing hydrogen into the biomass coal slurry to carry out a reaction under a pressure of 15 to 25 MPa to finally obtain a bio-oil;

wherein, when the flowing medium is an oil, said preparing a biomass coal slurry comprises: firstly removing dust from the biomass powder and the coal powder, and premixing them with the catalyst and the vulcanizing agent to obtain a premix, and then mixing the premix with the oil; or directly mixing the biomass powder, the coal powder which is pulverized again to a median particle size of 30-50  $\mu\text{m}$ , and the catalyst with the oil; and wherein the biomass powder and the coal powder account for 60-70 wt % of the mass of the biomass coal slurry; and the liquefaction reaction is carried out under a temperature of 380-460° C.; or

wherein, when the flowing medium is water, said preparing a biomass coal slurry comprises: firstly removing dust from the biomass powder and the coal powder, and premixing them with the catalyst and the vulcanizing agent to obtain a premix, and then mixing the premix with water; or directly mixing the biomass powder, the coal powder which is pulverized again to a median particle size of 30-100  $\mu\text{m}$ , the catalyst, and the vulcanizing agent with water; wherein, the biomass powder

**45**

and the coal powder account for 55-65 wt % of the mass of the biomass coal slurry; and the liquefaction reaction is carried out under a temperature of 300-460° C.

**26.** The process according to claim 25, wherein, when the flowing medium is an oil, the biomass accounts for 20-30 wt % of the mass of the biomass coal slurry, and the coal powder accounts for 30-45 wt % of the mass of the biomass coal slurry; and when the flowing medium is water, the biomass accounts for 15-30 wt % of the mass of the biomass coal slurry, and the coal powder accounts for 35-50 wt % of the mass of the biomass coal slurry.

**27.** The process according to claim 25, wherein, the moisture content is controlled by drying and dehydrating under a temperature of 50-70° C. for a period of 3-5 h.

**28.** The process according to claim 25 wherein, said preparing a biomass coal slurry comprises controlling the biomass powder to have a bulk density of 300-500 kg/m<sup>3</sup>, and controlling the coal powder to have a bulk density of 1000-1200 kg/m<sup>3</sup> when the flowing medium is an oil and a bulk density of 1200-1300 kg/m<sup>3</sup> when the flowing medium is water.

**29.** The process according to claim 25, wherein, the grinding pulping lasts for 2-8 min.

**30.** The process according to claim 25, wherein, the coal is low rank coal; the oil is selected from the group consisting of hogwash oil, gutter oil, rancid oil, waste lubricating oil, waste engine oil, heavy oil, residual oil, washing oil, anthracene oil, coal tar, petroleum, bio-oil produced by the present process, and any combination thereof.

**31.** The process according to claim 25, wherein, in the biomass coal slurry the catalyst is present in an amount of 1-10 wt %, preferably 1-4 wt %, of the total mass of the biomass and coal; and the catalyst has a particle size of 5-500 µm.

**32.** The process according to claim 25, wherein, said introducing hydrogen comprises:

introducing a high-pressure hydrogen into the biomass coal slurry to prepare a reaction raw material mixture, wherein the high-pressure hydrogen and the biomass coal slurry have a volume ratio of (600-1500):1; and heating the reaction raw material mixture to 320-450° C.

and feeding it into a slurry bed reactor to undergo

**46**

liquidation, cracking and hydrogenation reactions, and simultaneously introducing a cold hydrogen into the slurry bed reactor by controlling the slurry bed reactor to have a total gas velocity of 0.02-0.2 m/s, preferably 0.05-0.08 m/s;

wherein, the high-pressure hydrogen has a pressure of 13-27 MPa, and the cold hydrogen has a temperature of 60-135° C.

**33.** The process according to claim 32, wherein, said introducing the high-pressure hydrogen into the biomass coal slurry comprises two steps of:

firstly, introducing a high-pressure hydrogen into the biomass coal slurry till the volume ratio of the high-pressure hydrogen to the biomass coal slurry is (50-200):1, and heating the biomass coal slurry to 200-350° C., and

secondly, introducing a high-pressure hydrogen into the biomass coal slurry.

**34.** The process according to claim 32, wherein, the catalyst stored in the slurry bed reactor is controlled in an amount of 5-30 wt % of the mass of liquid phase in the slurry bed reactor.

**35.** The process according to claim 25, wherein, the liquefaction reaction lasts for 30-90 min when the flowing medium is an oil, and lasts for 30-60 min when the flowing medium is water.

**36.** The process according to claim 25, wherein, the catalyst comprises:

amorphous alumina loading a first active component, or biomass charcoal loading a first active component, wherein the first active component is selected from the group consisting of oxides of metals of group VIB, group VIIIB or group VIII, and any combination thereof in the periodic table of elements.

**37.** The process according to claim 25, wherein, the catalyst further comprises:

amorphous FeOOH, and/or biomass charcoal loading a second active component, wherein the second active component is selected from the group consisting of oxides of Mo, W, Fe, Co, Ni, Pd, and any combination thereof.

\* \* \* \* \*